



US005145487A

**United States Patent** [19]**Haney et al.**[11] **Patent Number:** **5,145,487**[45] **Date of Patent:** **Sep. 8, 1992**

[54] **METHODS AND COMPOSITIONS TO  
ENHANCE STAIN RESISTANCE OF CARPET  
FIBERS USING SULFONATED AROMATIC  
CONDENSATES**

[75] Inventors: **Dale A. Heney, Midlothian; Paul W. Harris; Charles J. Cole, both of Chester; Daniel J. Corcoran, Jr., Richmond, all of Va.**

[73] Assignee: **Allied-Signal Inc., Morris Township, N.J.**

[21] Appl. No.: **818,475**

[22] Filed: **Jan. 6, 1992**

**Related U.S. Application Data**

[60] Continuation of Ser. No. 399,106, Aug. 28, 1989, abandoned, which is a division of Ser. No. 361,671, Jun. 1, 1989, which is a continuation of Ser. No. 101,652, Sep. 28, 1987, abandoned.

[51] Int. Cl.<sup>5</sup> ..... **C09B 67/00; D06M 15/41;**  
D06M 101/34

[52] U.S. Cl. ..... **8/557; 8/560;**  
**8/589; 8/623; 8/115.56; 8/924; 8/929**

[58] Field of Search ..... **8/557, 560, 589**

[56]

**References Cited****U.S. PATENT DOCUMENTS**

|           |         |                       |         |
|-----------|---------|-----------------------|---------|
| 3,387,913 | 6/1968  | Tigler et al. ....    | 8/546   |
| 3,576,588 | 4/1971  | Wilson ....           | 8/534   |
| 3,652,199 | 3/1972  | Leung ....            | 8/629   |
| 4,592,940 | 6/1986  | Blyth et al. ....     | 252/8.7 |
| 4,619,853 | 10/1986 | Blyth et al. ....     | 428/95  |
| 4,680,212 | 7/1987  | Blyth et al. ....     | 428/97  |
| 4,780,099 | 10/1988 | Greschler et al. .... | 8/115.6 |
| 4,879,180 | 11/1989 | Blyth et al. ....     | 428/395 |

*Primary Examiner*—A. Lionel Clingman

[57]

**ABSTRACT**

This invention relates to improved methods and compositions to enhance stain resistance of carpet fiber. The improved methods relate to a continuous aftertreatment for dyed carpet fabric and to two-step processes, either batch-batch, batch-continuous or continuous-continuous. The improved compositions are used in the processes to enhance stain resistance of carpet or carpet fiber and to overcome various prior drawbacks, such as, yellowing, oxidation and durability to cleaning. The sulfonated aromatic condensates are used to enhance stain resistance, and can be combined with fluorocarbon compounds for soil resistance, thiocyanates, and/or salts having divalent cations, such as magnesium sulfate. Also various dispersing agents, buffering acids and sequestering agents are disclosed.

**8 Claims, No Drawings**

**METHODS AND COMPOSITIONS TO ENHANCE STAIN RESISTANCE OF CARPET FIBERS USING SULFONATED AROMATIC CONDENSATES**

**BACKGROUND OF THE INVENTION**

This application is a continuation of application Ser. No. 399,106 filed Aug. 28, 1989, now abandoned, which is a continuing application (divisional) of copending application Ser. No. 361,671, filed Jun. 1, 1989, which is a continuation of Ser. No. 101,652 filed Sep. 28, 1987, now abandoned.

This invention is related to improved methods and compositions to enhance stain resistance of carpet fibers. Sulfonated aromatic condensates alone in a new process or in combination with other compounds are used to improve stain resistance. Related technology is disclosed in commonly assigned, copending applications Ser. No. 889,705 filed Jul. 28, 1986, on sulfonated benzotriazoles and Ser. No. 074,487 filed Jul. 23, 1987, on sulfonated aromatic formaldehyde condensates, such as diphenyl ether condensates.

The following terms are defined for use in this specification.

By sulfonated aromatic condensate (s.a.c.) is meant any condensate of an aromatic compound whether sulfonated prior to or after condensation, particularly sulfonated aromatic formaldehyde condensate (s.a.f.c.), effective to enhance stain resistance of fiber or carpet fabric.

By thiocyanate is meant any salt, organic or inorganic, containing a cation and the thiocyanate anion.

By fluorocarbon is meant those fluorocarbon compounds effective to improve the antisoiling properties of fiber or carpet fabric.

By ICP is meant index of crystalline perfection, a measured indication of the internal crystal structure of the polymer in an oriented fiber. High ICP indicates an open crystalline internal structure, easily dyeable polymer fiber.

By nylon is meant the polyamide family of polymers, nylon 6, nylon 6,6, nylon 4, nylon 12 and the other polymers containing the



structure along with the  $[\text{CH}_2]_x$  chain.

By carpet fabric is meant carpet fiber or yarn which has been typically tufted, woven, or otherwise constructed into fabric suitable for final use in home furnishings, particularly as floor covering.

By fiber is meant continuous filament of a running or extremely long length or cut or otherwise short fiber known as staple. Carpet yarn may be made of multiple continuous filaments or spun staple fiber, both typically pretextured for increased bulk.

By salt having a divalent cation is meant any such salt effective to enhance stain resistance of fiber, particularly high ICP nylon fiber, when combined with an effective amount of a s.a.c.

By dispersing agent is meant any chemical compound or combination of chemical compounds effective to make stable, relatively nonprecipitating, noncoagulating mixtures of other chemical compounds.

By sequestering agent is meant any chelating agent which is effective in sequestration, which is the suppression

of certain properties of a metal without removing it from the system or phase. To be practical, the sequestering agent must not cause any undesirable change that would render the system unsuitable for its intended purpose. Chelation produces sequestration mainly by reducing the concentration of free metal ion to a very low value by converting most of the metal to a soluble chelate that does not possess the properties to be suppressed.

10 A chelating agent is a compound containing donor atoms that can combine by coordinate bonding with a single metal atom to form a cyclic structure called a chelation complex or, simply, a chelate. Because the donor atoms are connected intramolecularly by chains of other atoms, a chelate ring is formed for each donor atom after the first which coordinates with the metal. The above is from Volume 5, beginning page 339, of the Kirk-Othmer Encyclopedia of Chemical Technology (John Wiley & Sons), 1979, hereby incorporated by reference to p. 367.

15 It is known to use sulfonated aromatic formaldehyde condensates ("s.a.f.c.'s) in the yarn finish (during or after fiber quenching) to improve stain resistance of carpet fiber, see U.S. Pat. No. 4,680,212, in the dye bath for the same purpose, see U.S. Pat. No. 4,501,591 or incorporated into the fiber for the same purpose, see U.S. Pat. No. 4,579,762. All three above U.S. patents are hereby incorporated by reference, *in toto*. Use of fluorocarbon to improve both stain and soil resistance 20 in combination with s.a.f.c.'s is also taught in U.S. Pat. No. 4,680,212, column 5. Other useful fluorocarbons for antisoiling are taught in commonly assigned U.S. Pat. Nos. 4,192,754; 4,209,610; 4,414,277; 4,604,316; 25 4,605,587 all also hereby incorporated by reference, *in toto*.

30 It is known to use thiocyanates, such as ammonium thiocyanate, at different process conditions as "assists" during dyeing for various purposes. See U.S. Pat. No. 3,652,199; 3,576,588; 3,387,913; 2,899,262; and 2,615,718 all hereby incorporated by reference, *in toto*.

35 Use of salts containing a divalent cation, such as magnesium sulfate, with s.a.f.c.'s to improve wet fastness is known in U.S. Pat. No. 3,790,344, hereby incorporated by reference, *in toto*. Also see page 48 of a textbook by Rosen, M. J., *Surfactants & Interficial Phenomena* (Wiley, 1978).

40 It is also known generally to use acid, including citric acid to buffer a dye bath and to use dispersing agents and/or sequestering agents to stabilize aqueous formulations of chemicals.

45 Nylon carpets may be permanently discolored or stained by certain artificial colorants, such as food dyes, or oxidizing agents, such as acne preparations containing benzoyl peroxide. S.A.C.'s, applied to the fiber to provide an ionic barrier to food colorants, make the fiber more stain resistant, but are not effective against oxidizing agents. Furthermore, many of the s.a.c.'s used commercially for the preparation of "stain resistant" carpets are themselves, susceptible to oxidation upon exposure to light and ozone. This results in a yellowing of the s.a.c. and subsequent destruction. This has a major impact on the carpet properties. The yellow color of the s.a.c. results in a perceptible shift in the color of the carpet. Destruction of the s.a.c. results in a loss of the stain resistance properties of the carpet.

50 Use of fluorocarbon compound treated nylon fiber in carpet fabric inhibits wetting of the fiber surfaces which

also inhibits any staining agent from being adsorbed onto or absorbed into the fiber. This surface wetting inhibition can be insufficient when the staining agent is dropped on the carpet with enough force to break the surface energy of the fluorocarbon surface barrier or not cleaned from the carpet and left in contact with fibers for extended time. Carpet treated with compositions containing s.a.c.'s must not interfere with the anti-soiling properties of the fluorocarbon.

Application of s.a.c. to the carpet fabric must be effective, economical, and compatible to both untreated and fluorocarbon treated fiber, and to both continuous dyeing and Beck or batch dyeing. The same is true of any s.a.c. application formulation. The s.a.c. formulation must achieve effective penetration into the carpet fabric. Exhaustion of the individual active chemical components of any s.a.c. formulation must also be effective if not complete.

Certain nylon polymer fibers have very open internal crystal structure, namely high ICP polymer fiber, which require large amounts of s.a.c. to impart an effective degree of stain resistance. High ICP polymers are usually the result of high temperature saturated steam heat setting processes.

Some prior compositions and methods are only marginally acceptable regarding durability of the stain resistance when the carpet is steam cleaned with a detergent at a high pH.

#### SUMMARY OF THE INVENTION

This invention is several interrelated embodiments wherein the several new s.a.c. application formulations are used in the several new application processes. First described is a continuous aftertreatment for dyed nylon carpet fabric, using several combinations of chemical compositions to apply a s.a.c.. Then the two-step process of treating carpet fabric with a s.a.c., still using the continuous aftertreatment as the second step is described. This includes batch (or beck)-continuous and continuous-continuous two-step treatment. The combination of s.a.c. and the thiocyanates, and with various added chemicals, to improve resistance of dye and s.a.c. on the fiber to oxidation is next described. Then the method to improve stain resistance of nylon fiber, particularly high ICP fiber, using s.a.c., thiocyanate and a salt having a divalent cation and with additional added chemicals is described. The method to improve light induced yellowing of s.a.c. treated fiber by buffering with citric acid or any acid with a sequestering agent is an embodiment described throughout and specifically at this point. Then the new two-step batch-batch process is described used with various formulations. Finally described is an improved method to exhaust thiocyanate at low pH.

The first embodiment of this invention is a method to continuously treat dyed nylon carpet fabric to impart improved resistance to staining comprising preheating the dyed carpet fabric with water at a temperature of between about 140° and 212° F. (60° and 100° C.) to a wet pick-up of above about 75% by weight, and a carpet temperature of between about 130° and 210° F. (54.4° and 99° C.), then extracting the water from the carpet fabric to a wet pick-up of between about 30 to 190% by weight, then applying an aqueous solution of an effective amount of a sulfonated aromatic condensate to the carpet fabric at a pH of between about 1.5 to 5.5, at a concentration of between about 0.25 and 40 grams of solids of said condensate per liter of aqueous solution,

at a wet pick-up between 200 and 650% by weight, an aqueous solution liquor of between about 140° and 212° F. (60° and 100° C.) to achieve a carpet fabric temperature between about 130° and 210° F. (54.4° and 99° C.), then holding the carpet in the aqueous solution for between about 0.5 to 90 seconds at a temperature above 130° F. (54.4° C.). The carpet fabric can subsequently be washed in water. The preferred sulfonated aromatic condensate has been condensed with formaldehyde. 10 The method of extracting can be by applying vacuum to the wet carpet fabric or by squeezing the wet carpet fabric with a pair of rollers. The preferred concentration of the condensate is between about 0.25 and 10 grams per liter of aqueous solution. The preferred wet 15 pick-up of the aqueous solution is between about 300 and 600% by weight. When the aqueous solution is applied by pressurized contact with the carpet fabric, the wet pick-up preferred maximum is 450%. When the aqueous solution is applied by spray, the preferred wet pick-up minimum is 400%. It is preferred that the carpet fabric be held in the aqueous solution for between about 2 and 30 seconds. The preferred wet pick-up after extracting is between about 50 and 150% by weight. The sulfonated aromatic formaldehyde condensate can 20 be formed by condensation of formaldehyde with one or more phenols. At least one of the phenols can be phenol sulfonic acid or the alkali metal salt thereof. It is preferred that one of the phenols be dihydroxy aromatic diphenylsulfone. It is most preferred that the condensate be formaldehyde condensed with the alkali metal salt of para-phenol sulfonic acid and with 4,4'-diphenylsulfone. The beginning dyed carpet fabric of this process may also comprise an effective amount of a fluorocarbon compound intended to improve resistance to 25 soiling of the carpet. The preferred amount of fluorocarbon present is an amount of from about 0.05 to 0.4% by weight of the fabric. The fluorocarbon can contain perfluoroalkyl radical or can be a mixture of fluorinated pyromellitate oligomers. A more preferred fluorocarbon is a mixture of pyromellitate oligomers formed by two reactions, first, the reaction of pyromellitic dianhydride with the fluorinated alcohol, and second, the reaction product of the first reaction further reacted with epichlorohydrin. Another preferred fluorocarbon is a 30 reaction product of a perfluoroalkyl alcohol or amide with a suitable anhydride or isocyanate. Another more preferred fluorocarbon is a reaction product of N-ethyl perfluorooctyl-sulfoamido ethanol with toluene diisocyanate. The aqueous solution of this method may also contain an effective amount of a thiocyanate. The thiocyanate cation may be ammonium, sodium, potassium, copper, zinc, ferrous, ferric, methyl or phenyl, preferred is ammonium. The aqueous solution of this method may also contain an effective amount of a dispersing agent. The dispersing agent can be a condensed naphthalenic salt, alkyl sulfosuccinate or mixtures thereof. The preferred dispersing agent is a mixture of a sodium salt of condensed naphthalenic sulfonic acid and di-isobutyl sulfosuccinate. The aqueous solution of this 35 method may also contain an effective amount of a salt having a divalent cation. The preferred salt is calcium, magnesium, zinc, or ferrous chloride, sulfate or phosphate wherein the most preferred is magnesium sulfate. The preferred aqueous solution would contain the combination of a sulfonated aromatic condensate, a salt containing a divalent cation, a thiocyanate, and a dispersing agent, the most preferred combination would be wherein the condensate is formaldehyde condensed 40 45 50 55 60 65

with the alkali metal salt of para-phenol sulfonic acid and with 4,4'-diphenolsulfone, the thiocyanate is ammonium thiocyanate, the divalent cationic salt is magnesium sulfate and the preferred dispersing agents are di-isobutyl sulfosuccinate and the sodium salt of condensed naphthalene sulfonic acid in a mixture. The preferred carpet fabric would comprise a fiber treated with a fluorocarbon. The fluorocarbon is a mixture of pyromellitate oligomers formed by two reactions, first the reaction of pyromellitic dianhydride with a fluorinated alcohol, second, the reaction product of the first reaction further reacted with epichlorohydrin. The amounts of the fluorocarbon present on the carpet fabric used in the method is an amount between about 0.05 and 0.4% by weight of the fabric, the magnesium sulfate can be present in the aqueous solution of the method in an amount between about 0.05 and 0.8% on the weight of the fabric, the ammonium thiocyanate can be present in an amount in about 0.03 to 1% on the weight of the fabric, the sulfonated aromatic condensate can be present in an amount of between about 0.15 and 7.5% on the weight of the fabric, the dialkyl sulfosuccinate can be present in an amount of between 0 and 6 parts by weight to the parts by weight of the sulfonated aromatic condensate and the sodium salt of the condensed naphthalenic acid can be present in an amount between about 0 and 3 parts by weight to parts by weight of the sulfonated aromatic condensate. The preferred amounts of the compounds are about 0.05 and 0.4% by weight of the fabric of the fluorocarbon, between about 0.08 and 0.4% on the weight of the fabric of the magnesium sulfate, between 0.15 and 0.7% on the weight of the fabric of the ammonium thiocyanate and between about 0.15 and 1.5% on the weight of the fabric of the sulfonated aromatic condensate with the dialkyl sulfosuccinate being present in an amount between 0 and 2.5 parts by weight to the parts by weight of the sulfonated aromatic condensate and the sodium salt of the condensed naphthalenic acid being present in an amount between 0 and 2 parts by weight to parts by weight of the sulfonated aromatic condensate. In order to improve yellowing of the carpet fabric, any of the above aqueous solutions can be buffered with an effective amount of citric acid or any other acid with a sequestering agent. The preferred aqueous solution is buffered with an amount of citric acid between 0.3 and 5.5 grams per liter of aqueous solution.

A two-step process embodiment of this invention uses the aftertreatment process described above but, preceding the initial preheating step of that aftertreatment a portion of the effective amount of the sulfonated aromatic condensate is added during dyeing of the carpet fabric and another portion is added in the above-described aftertreatment so that the portion of sulfonated aromatic condensate added during dyeing and the portion added after dyeing combined make an amount effective to make the carpet resistant to staining. Surprisingly, the effective amount added in portions (as described above and in Example 1) is substantially less than the effective amount necessary if added either only during dyeing or only after dyeing. An effective amount of the salt having a divalent cation can be added during the dyeing so that the s.a.c. exhausts onto the fiber at the possibly higher pH and so that the stain resistance of the nylon fiber in the carpet fabric, especially an easily dyed nylon fiber having a high index of crystalline perfection and having a very open internal crystal polymer structure, is enhanced and durability

steam cleaning of the stain resistance is enhanced, or the effective amount of sulfonated aromatic condensate is lower to achieve the same level of stain resistance. The divalent salt again can be calcium, zinc, magnesium or ferrous sulfate, chloride or phosphate. The preferred salt is magnesium sulfate. The preferred amounts of sulfonated aromatic condensate added during dyeing and after dyeing are between about 0.05% on the weight of the fiber to 0.5% on the weight of the fiber during dyeing, an additional 0.05% on the weight of the fiber to 7.5% on the weight of the fiber after dyeing. Also, the preferred amounts of magnesium sulfate are 0.03 to 1% on the weight of the fiber added to the dye-bath and 0.05 to 1% on the weight of the fiber added after dyeing. The carpet fabric used in the method can comprise a fluorocarbon present dyeing. The fluorocarbon again can contain perfluoroalkyl radical or a mixture of fluorinated pyromellitic oligomers. The preferred fluorocarbon is a mixture of pyromellitic oligomers formed by two reactions, first, the reaction of pyromellitic dianhydride with a fluorinated alcohol, and second, the reaction product of the first reaction further reacted with epichlorohydrin. The preceding dyeing step can either be a continuous dyeing operation or it can be batch or beck dyeing. The beck dyeing can be done in the presence of an effective amount of a salt having a divalent cation so that the stain resistance of the carpet fabric is enhanced. The preferred amount of magnesium sulfate in the dyebath is an amount between 0.2% on the weight of the fiber to 5% on the weight of the fiber.

Another method to improve stain resistance of nylon or wool fiber comprises treating the fiber with a combination of an effective amount of each of a sulfonated aromatic condensate and a thiocyanate, whereby improved resistance to oxidation to ozone or by other strong oxidizing agents such as benzoyl peroxide is imparted to the s.a.c. and the dye on the fiber. The preferred fiber is carpet fiber, the preferred aromatic condensate is sulfonated aromatic formaldehyde condensate formed by condensation with one or more phenols. At least one of the phenols can be a phenol sulfonic acid or the alkali metal salt thereof. Or at least one of the phenols can be a sulfone. The sulfone can be a dihydroxy aromatic diphenolsulfone. The preferred condensate is formaldehyde condensed with a alkali metal salt of para-phenol sulfonic acid and with 4,4'-diphenolsulfone. This method of improving stain resistance of nylon or wool fiber using a thiocyanate with the sulfonated aromatic condensate can use a thiocyanate selected from the group consisting of ammonium, sodium, potassium, copper, zinc, ferrous, ferric, methyl and phenyl thiocyanate. The most preferred is ammonium thiocyanate. The dispersing agent can be added to the mixture applied to the fiber in this method also. The dispersing agent can be selected from the group consisting of condensed naphthalenic salt, an alkyl sulfosuccinate or a mixture thereof. The preferred dispersing agent is a mixture of the sodium salt of condensed naphthalene sulfonic acid and di-isobutyl sulfosuccinate. The preferred amounts used in this method are between about 0.05 and 10% on weight of the fiber of the sulfonated aromatic condensate, between about 0.1 and 5% on weight of the fiber of the thiocyanate and the sodium salt of the condensed naphthalenic sulfonic acid is added in an amount between 0 and 3 parts by weight by parts by weight of the sulfonated aromatic condensate and the di-isobutyl sulfosuccinate is added in amount

between 0 and 6 parts by weight to the parts by weight of sulfonated aromatic condensate.

Yet another method of improving stain resistance of nylon fiber, particularly fiber having a high index of crystalline perfection, for carpet comprises treating the fiber with a combination of an effective amount each of a sulfonated aromatic condensate, thiocyanate and salt having a divalent cation. The sulfonated aromatic condensate can be a condensate with formaldehyde, can further be formed by the condensation of formaldehyde with one or more phenols and at least one of the phenols can be phenol sulfonic acid and the alkali metal salt thereof or sulfone. The preferred condensate is formaldehyde condensed with a alkali metal salt of para-phenol sulfonic acid and with 4,4'-diphenolsulfone. The preferred thiocyanate is ammonium thiocyanate but the thiocyanate can be ammonium, sodium, potassium, copper, zinc, ferrous, ferric, methyl or phenyl. The preferred salt is magnesium sulfate but the salt can be calcium, magnesium or ferrous chloride, sulfate or phosphate. The fiber treated can comprise an effective amount of the fluorocarbon compound intended to enhance soil resistance of the fiber. The preferred fluorocarbon is a mixture of pyromellitate oligomers formed by two reactions, first the reaction of pyromellitic dianhydride with a fluorinated alcohol and second a reaction product of the first reaction further reacted with epichlorohydrin. A dispersing agent can be added to the combination used to treat the fiber in this method. Dispersing agents can be condensed naphthalenic salt or an alkyl sulfosuccinate or a mixture thereof. The preferred amounts are between 0.15 and 7.5% on weight of the fiber of the sulfonated aromatic condensate between 0.15 and 1% on weight of the fabric of the thiocyanate, between 0.05 and 0.8% on weight of the fabric of the sulfonated aromatic condensate, between about 0.1 and 5% on weight of the fiber of the thiocyanate and the divalent cation salt, and between 0.05 and 0.4% on the weight of the fabric of the fluorocarbon present on the fiber before dyeing. As above the condensate and thiocyanate can be buffered with an effective amount of citric acid or any acid with a sequestering agent so light induced yellowing of the stain resistant fiber is reduced.

A method of improving light induced yellowing of stain resistant nylon in fiber treated with an effective amount of sulfonated aromatic condensate from an aqueous solution comprises using an effective amount of citric acid or any acid with a sequestering agent to buffer the aqueous solution containing the sulfonated aromatic condensate for treating the fiber at a pH between about 1 and 5.5.

Another two-step treatment is a method to dye and treat in two steps (both batch or beck) nylon carpet fabric to impart improved resistance to staining comprising dyeing in a first step in dyed carpet fabric in a dyebath liquor in the presence of a portion of an effective amount of a sulfonated aromatic condensate in an aqueous solution at an elevated temperature then removing the dyebath liquor from the dyed carpet fabric then rinsing the dyed carpet fabric then applying in a second step another portion of an effective amount of a sulfonated aromatic condensate in an aqueous solution to the dyed carpet fabric at a pH between 1.5 to 5.5 at a liquor temperature between 110° and 195° F. (60° and 91° C.) so that the total of both portions of effective amounts to effect stain resistance of sulfonated aromatic condensate in both steps is less than total effective amount necessary if applied in either the first dye step

solely or in a subsequent application step solely or so that a more effective degree of stain resistance of the carpet fabric is achieved at the same total of effective amounts of sulfonated aromatic condensate in said two steps as compared to the same amount in if applied either step solely. The dyeing conditions in the first step are a liquor to fabric ratio of about 10:1 to 100:1 at a temperature of 158° to 212° F. (70° to 100° C.) for 15 to 90 minutes. Preferred conditions for the second step are a liquor to fabric ratio of about 10:1 to 100:1 for a period of about 5 to 60 minutes. The carpet fabric can be also rinsed subsequent to the second step. The sulfonated aromatic condensate can be condensed with formaldehyde. The sulfonated aromatic formaldehyde condensate can be formed by condensation of formaldehyde with one or more phenols. The phenols can be phenol sulfonic acid or the alkali metal salt thereof. Or the phenol can be dihydroxy aromatic diphenol sulfone. The preferred condensate is formaldehyde condensed with alkali metal salt of para-phenol sulfonic acid and with 4,4'-diphenolsulfone. Here again the dyed carpet fabric can comprise an effective amount of a fluorocarbon intended to improve the resistance of soiling of the carpet. The preferred amount of the fluorocarbon is present in an amount of from about 0.05 to 0.4% by weight on weight of the fabric. The fluorocarbon can contain perfluoroalkyl radical or a mixture of fluorinated pyromellitate oligomers. The fluorocarbon can be the reaction product of a perfluoroalkyl alcohol or amide with a suitable anhydride or isocyanate. The fluorocarbon can be the reaction product of N-ethyl perfluoroctylsulfoamide ethanol with toluene diisocyanate. The preferred fluorocarbon is a mixture of pyromellitate oligomers formed by two reactions, first, the reaction of pyromellitic dianhydride with a fluorinated alcohol, and second, the first reaction product is further reacted with epichlorohydrin. The second step aqueous solution can also contain an effective amount of a thiocyanate such as ammonium, sodium, potassium, copper, zinc, ferrous, ferric, methyl or phenyl thiocyanate. The preferred thiocyanate is ammonium thiocyanate. The aqueous solution of either or both application steps can also contain an effective amount of dispersing agent such a condensed naphthalenic salt, an alkyl sulfosuccinate or a mixture thereof. The preferred dispersing agent is a mixture of the sodium salt of condensed naphthalene sulfonic acid and di-isobutyl sulfosuccinate. The aqueous solutions of both steps of liquor to fabric ratio of about 10:1 to 100:1 for a period of about 5 to 60 minutes. The carpet fabric can be also rinsed subsequent to the second step. The sulfonated aromatic condensate can be condensed with formaldehyde. The sulfonated aromatic formaldehyde condensate can be formed by condensation of formaldehyde with one or more phenols. The phenols can be phenol sulfonic acid or the alkali metal salt thereof. Or the phenol can be dihydroxy aromatic diphenol sulfone. The preferred condensate is formaldehyde condensed with alkali metal salt of para-phenol sulfonic acid and with 4,4'-diphenolsulfone. Here again the dyed carpet fabric can comprise an effective amount of a fluorocarbon intended to improve the resistance of soiling of the carpet. The preferred amount of the fluorocarbon is present in an amount of from about 0.05 to 0.4% by weight on weight of the fabric. The fluorocarbon can contain perfluoroalkyl radical or a mixture of fluorinated pyromellitate oligomers. The fluorocarbon can be the reaction product of a perfluoroalkyl alcohol or amide with a suitable

anhydride or isocyanate. The fluorocarbon can be the reaction product of N-ethyl perfluoroctylsulfoamideo ethanol with toluene diisocyanate. The preferred fluorocarbon is a mixture of pyromellitate oligomers formed by two reactions, first, the reaction of pyromellitic dianhydride with a fluorinated alcohol, and second, the first reaction product is further reacted with epichlorodrin. The second step aqueous solution can also contain an effective amount of a thiocyanate such as ammonium, sodium, potassium, copper, zinc, ferrous, ferric, methyl or phenyl thiocyanate. The preferred thiocyanate is ammonium thiocyanate. The aqueous solution of either or both application steps can also contain an effective amount of dispersing agent such a condensed naphthalenic salt, an alkyl sulfosuccinate or a mixture thereof. The preferred dispersing agent is a mixture of the sodium salt of condensed naphthalene sulfonic acid and di-isobutyl sulfosuccinate. The aqueous solutions of both steps of this invention can also contain an effective amount of salt having divalent cation such calcium, magnesium or ferrous chloride, sulfate or phosphate, preferably magnesium sulfate. The preferred amounts of this method would be having the fluorocarbon present in an amount of 0.05 and 0.4% by weight of the fabric, magnesium sulfate present in an amount of between 0.25 and 4% on the weight of the fabric, ammonium thiocyanate present in an amount between 0.03 and 1% on the weight of the fabric, the sulfonated aromatic formaldehyde condensate present in an amount between 0.15 and 7.5% on the weight of the fabric and the dialkyl sulfosuccinate present in an amount between 0 and 6 parts by parts by weight of the sulfonated aromatic condensate and the sodium salt of a condensed naphthalenic acid is present in an amount between 0 and 3 parts by weight by parts by weight of sulfonated aromatic condensate. The more preferred amounts are where the fluorocarbon is present in an amount of between about 0.05 and 0.4% on the weight of the fabric, the magnesium sulfate is present in an amount between 0.25 and 1.5% on the weight of the fabric, ammonium thiocyanate is present in an amount between 0.05 and 0.75% on the weight of the fabric, sulfonated aromatic formaldehyde condensate is present in an amount between 0.15 and 2.0% on the weight of the fabric and the dialkyl sulfosuccinate is present in an amount between 0 and 2.5 parts by weight to the parts by weight of the sulfonated aromatic condensate and the sodium salt of a condensed naphthalenic acid is present in an amount between 0 and 2 parts by weight to the parts by weight of the sulfonated aromatic condensate. Here again aqueous solution can be buffered with an effective amount of citric acid or any other acid with a sequestering agent to improve the yellowing of the carpet fabric.

Finally, in the last embodiment of this invention a method of improving exhaustion of a water soluble thiocyanate onto polyamide fiber comprising contacting the fiber with an effective amount of the thiocyanate at a pH between about 1 and 5 wherein the fiber has improved resistance to fading of dye, due to strong oxidizing agents such as benzoyl peroxide or ozone, the dye being present in or on the fiber, is disclosed. The thiocyanate can be ammonium, sodium, potassium, copper, zinc, ferrous, ferric, methyl or phenyl thiocyanate. The preferred pH of the method is between 1 and 4. The preferred amount of thiocyanate is between about 0.1 and 6% on the weight of the fiber of the thiocyanate, present in or on the fiber after dyeing. The method

improves exhaustion so that between about 0.1 and about 12% on the weight of the fiber of the thiocyanate is present during the contacting and at least 50% of the thiocyanate present during the contacting is exhausted onto or into the fiber. The preferred thiocyanate is ammonium thiocyanate. The thiocyanate can be contacted with the fiber in the dyebath or after dyeing of the fiber. The fiber being treated can comprise an effective amount of a fluorocarbon to inhibit soiling of the fiber and a sulfonated aromatic condensate can be present either on the fiber or with the thiocyanate. The various fluorocarbons are as described above. An effective amount of citric acid or any acid with a sequestering agent can also be used to buffer for the condensate and thiocyanate to the desired pH for this same anti-yellowing effect. It is preferred to have between about 0.1 and 12% thiocyanate on the weight of the fiber and between about 0.05 and 0.4% fluorocarbon on the weight of the fiber.

## PREFERRED EMBODIMENTS

### Continuous Aftertreatment Process

This process is intended to continuously treat nylon carpet fabric with sulfonated aromatic condensate formulations, for instance on a continuous dye range after steaming but before washing; or piece (or beck) dyed carpets may be continuously treated in a similar fashion by treating in-line on the wet goods dryer range prior to the dryer. Equipment could be a spray header(s), or the equivalent, for the heated water across the moving carpet fabric with vacuum extractors below or a set of squeeze rolls to remove the water, followed by spray headers for the treatment liquor with a catch pan underneath. An alternative to spray application is use of a pressurized applicator, such as a Kusters Fluidyer, which presses the carpet into contact with a narrow slot in a conduit containing treatment liquor under pressure.

The prior art describes the application of similar sulfonated aromatic formaldehyde condensates by a beck (piece) aftertreatment and a continuous manner along with dyestuffs and subsequent steaming. The continuous process of this invention has economical advantages over the beck aftertreatment process by approximately 4 cents per pound of fiber produced as finished carpet (at equal levels of the stain resist agent on the fiber). The continuous aftertreatment process of this invention has the following advantages over the known prior art processes:

(a) Post dyeing process. Process conditions are optimized for the "exhaustion" of the sulfonated aromatic formaldehyde condensate onto the fiber. These conditions are not necessarily compatible with the dyeing process. Since the treatment process occurs after dyeing, there is no interference with the dyeing process. Prior art concurrent (with dyes) processes generally result in poorer dyeing quality, a loss in dye yield and an effect of the dyed shade of the carpet.

(b) More versatile. The process of this invention is applicable to both continuously dyed solid or multi-color patterns with the same process conditions. Furthermore, the process is also applicable to continuously aftertreating piece (or beck) dyed goods at the wet goods dryer.

The process involves the general principle of first, preheating the carpet with heated water followed by hydroextraction and the application of an aqueous solution of the sulfonated aromatic formaldehyde condensate.

sate, for which there are specific ranges of pH, concentration, wet pick-up (w.p.u.) and temperatures. This is followed by a dwell period at which the carpet is either held at temperature or is allowed to radiant cool prior to washing the carpet. Prior to the treatment, the carpet has already been dyed by either beck or continuous methods. For beck-dyed carpets the treatment process is at the wet goods dryer and for continuously-dyed carpets the treatment process is in-line after steaming and prior to the final washing step.

The process, in more detail, involves preheating the dyed carpet with hot water followed by hydroextraction by either squeeze or vacuum methods to a wet pick-up of 30 to 190%. The conditions of the preheating process are established to achieve a carpet temperature of 130° to 210° F. (54.4° to 99° C.) prior to the treatment stage. The conditions of the preheating process are generally using 200% w.p.u. to total saturation with water at 140° to 212° F. (60° to 100° C.). As an addition in the continuous dyeing process, this also gives the carpet a washing prior to application of the treatment solution which aids the carpet's receptiveness to the stain resist agent. The treatment solution is an aqueous solution of the sulfonated aromatic condensate at a 0.25 to 40 grams per liter concentration and a pH of 1.5 to 5.5. The treatment solution is applied at 200 to 600% w.p.u. add-on and a temperature of 140° to 212° F. (60° to 100° C.). The resulting temperature of the carpet must be in the 130° to 210° F. (54.4° to 99° C.) range for the treatment to be effective. It is preferred to keep the difference in carpet fabric temperature between pre-treating and application to a minimum. Following the application of the treatment liquor, it is necessary to either maintain the carpet at the application temperature for at least 0.5 to 30 seconds or allow it to radiantly cool to no less than 130° F. (54.4° C.).

The equipment used for the application of the treatment liquor may be either spray or contact (e.g. Kusters Fluidyer) in nature. The contact method is preferred since it is easier to achieve 100% penetration of the treatment. Spray processes are adequate provided that the solution penetrates to the back of the carpet, and will generally require additional mechanical considerations, such as a squeeze or "S" rollers to achieve complete penetration. Other application equipment may also be used as long as the process requirements of preheating, heated treatment and dwell time at temperature are satisfied. The preheating and/or extracting steps of this invention may be carried out on the previously existing equipment.

The practical significance of this invention is that it provides an economical and effective means to apply sulfonated aromatic formaldehyde condensates to impart stain resistance to dyed carpets. The process is 55 applicable to over 90% of all carpets treated with sulfonated aromatic formaldehyde condensates.

The continuous aftertreatment embodiment can also be the second step of another two-step process embodiment of this invention wherein an effective amount of the sulfonated aromatic condensate is added to a continuous dyebath or in batch or beck process for dyeing carpet fabric. The two-step process uses less overall amount sulfonated aromatic condensate for the same 60 effect level of stain resistance. Alternatively, the same total amount of sulfonated aromatic condensate can be used in the two-step process to achieve a higher level of stain resistance.

Certain nylon substrates (fiber) have very open internal structure (orientation of the polymer chains) which require very high amounts of the sulfonated aromatic condensate composition to impart a marketable degree 5 of stain resistance. Certain sulfonated aromatic condensate compositions cannot achieve a sufficient level of protection on these substrates, so they must be excluded. Also, the continuous aftertreatment method results in only moderate durability of the stain resistance properties to steam cleaning when a high pH 10 detergent is used.

The two-step application process has all of the advantages of the continuous aftertreatment process such as economics, etc. over one-step batch processes. It also 15 has unique advantages over the aftertreatment process alone and all other known continuous application processes for sulfonated aromatic condensates, such as using all of the sulfonated aromatic condensate in dye-bath (currently being practiced on a commercial scale).

20 The level of stain resistance imparted by a given total amount of the sulfonated aromatic condensate is substantially improved. The required add-on for a marketable level of stain resistance reduced by approximately 30% over aftertreatment and greater for other continuous processes, providing economical advantages. The process (with optimized sulfonated aromatic condensate composition for aftertreatment) yields marketable 25 levels of stain resistance on critical substrates described above using reasonable levels of the sulfonated aromatic condensate composition. The durability of the stain 30 resistance properties to steam cleaning (with and without a high pH detergent) is improved over the aftertreatment only process, yielding improved properties.

The two-step process involves the general principle 35 of applying a portion of the total sulfonated aromatic condensate composition to be applied in the standard dyebath with an appropriate amount of magnesium sulfate (magnesium sulfate, 0 to 0.35% on the weight of the fabric for each 1% on the weight of the fabric of the 40 sulfonated aromatic condensate). The balance of the total sulfonated aromatic condensate composition (with 0 to 0.35% of magnesium sulfate) is then applied as an aftertreatment. The amount of Epsom Salt required in both portions depends on the sulfonated aromatic condensate and the substrate being treated.

The dyebath composition is based on that typically 45 used for continuous dyeing. The appropriate amount of the sulfonated aromatic condensate composition (based on the optimum ratio and the total required for the 50 particular substrate) is added to the dyebath.

More specific examples of the processes are given in the following Examples.

#### Preferred Treatment Compositions

In addition to a sulfonated aromatic condensate other chemical compounds such as a thiocyanate are added to the formulation used to treat the carpet fabric to overcome oxidative yellowing of the sulfonated aromatic condensate, and to provide the resulting carpet with better resistance of the dyes to strong oxidizing agents, such as ozone or the benzoyl peroxide found in commercial anti-acne preparations. Also a salt containing a divalent cation is useful to improve exhaustion of the sulfonated aromatic condensate on high ICP polymer fibers. A dispersing agent(s) is usually necessary in the formulation to prevent precipitation or coagulation due to incompatibility of the components of the formulation for treatment and/or the components with a fluorocar-

bon treated carpet fabric. Acids are used to buffer the formulations. It has been discovered that citric acid or any acid with a sequestering agent creates an additional improvement in yellowing characteristics of sulfonated aromatic condensate treated fiber or fabric.

Ammonium thiocyanate and sulfonated aromatic condensates exhaust onto nylon fibers under comparable application procedures. The two products may be co-applied providing that the uptake of one material does not interfere with the other. Therefore, the selection of the sulfonated aromatic condensate is important. Some sulfonated aromatic condensates exhaust preferentially over ammonium thiocyanate. But to the contrary there was a synergistic effect of Intratex N (which is reported to be formaldehyde condensed with an alkali metal salt of para-phenol sulfonic acid and with 4,4'-diphenolsulfone) and ammonium thiocyanate on benzoyl peroxide spotting resistance.

An additional benefit of ammonium thiocyanate in the composition is as an antioxidant to prevent light induced yellowing of Intratex N. This combination was found to give a sufficient improvement (acceptable light-fastness) for beck applications, but was insufficient for continuous applications (although improved).

The combination of sequestering agents, such as EDTA and sodium hexametaphosphate, with Intratex N was found to result in some improvement in light induced yellowing, but did not yield completely acceptable results for the continuous application. Combination of Intratex N with citric acid (sequestering and antioxidant properties) also gave similar results. The combination of ammonium thiocyanate and citric acid was discovered to achieve the best results in the reduction of light induced yellowing for continuous application, showing virtually no yellowing. (Combinations of ammonium thiocyanate and other sequestering agents were not as effective.)

A novel dispersant system, using Tamol SN and Monawet MB-45 was developed to prepare a stable composition containing Intratex N, ammonium thiocyanate and citric acid in concentrated form for continuous applications. A new dispersant system was developed to prepare a stable concentrate containing Intratex N and ammonium thiocyanate for beck applications.

the copper, ferrous and ferric thiocyanates may have to be color compensated.

As dispersing agents any agent that is effective can be used, such as for any process formulation, the condensed naphthalenic salts, the alkyl sulfosuccinates, a mixture of them, and for batch process systems salts of polymeric carboxylic acid, and polyethylene glycol ethers.

As sequestering agents, the polyphosphates, such as sodium tripolyphosphate (STPP), aminocarboxylic acids, such as ethylenediamine tetraacetic acid (EDTA), hydroxycarboxylic acids, such as tartaric and citric acid, and the aminoalcohols, such as triethanolamine (TEA) are expected to be effective. See Kirk-Othmer Encyclopedia of Chemical Technology, supra.

#### EXAMPLE 1

On a commercial dyeing range Composition 1 was applied both in a two-step (continuous-continuous) and in a continuous aftertreatment only process to a normal and to a high ICP fiber carpet fabric. The normal fiber was in an 1186 denier Superba heat set textured yarn. The high ICP fiber was a 1700 denier textured yarn which was heat set by a proprietary Pharr process with a high heat history giving an ICP of 3.92 compared to normal ICP of about 3.8. Both fibers were previously treated with a spin finish containing a soil-release fluorocarbon as described in U.S. Pat. No. 4,604,316 and/or U.S. Pat. No. 4,192,754. The fabric was dyed gray. The prewash and treatment application was by spray just after the dryer but before the final wash on the continuous dye range. Following are the dyes and chemicals used in the continuous dyebath.

#### Control

35 0.135 g/l \*\* Nylanthrene<sup>1</sup> Orange RAR (liquid)  
 0.092 g/l Tectilon<sup>2</sup> Red 2B Liq.-50  
 0.052 g/l Telon<sup>3</sup> Blue B-AR (powder) (the above dyes  
 are the same for all dyebaths.)  
 40 3.0 g/l Alrowet<sup>2</sup> D-70 \*  
 1.0 g/l Chemcogen<sup>4</sup> DCG \*  
 0.5 g/l Defoamer AC (Fuller) \*  
 pH 5.5 with Acetic Acid  
 400% w.p.u. via Kuster Fluidyer  
 45 Steam in vertical steamer 5 to 6 minutes

#### "4% Dyebath"

(Order of addition to bath as listed.)  
 50 3.0 g/l Alrowet D-70  
 1.0 g/l Chemcogen DCG  
 0.5 g/l Defoamer AC (Fuller)  
 10.0 g/l Composition 1  
 1.25 g/l Epsom Salt (Magnesium Sulfate)  
 0.5 g/l Sequestrene<sup>2</sup> 30A \*  
 55 Dyes above  
 Approximately 1 g/l Ammonia to pH 5.5

#### "8% Dyebath"

(Order of addition to bath as listed.)  
 60 3.0 g/l Alrowet D-70  
 1.0 g/l Chemcogen DCG  
 0.5 g/l Defoamer AC (Fuller)  
 20.0 g/l Composition 1  
 2.5 g/l Epsom Salt (Magnesium Sulfate)  
 0.5 g/l Sequestrene 30A \*  
 Dyes above  
 Approximately 3 g/l Ammonia to pH 5.5

\*Same concentration of same s.a.c., N-1 has pH 7, N has pH 10.5.  
 \*Alrowet D-70 is dioctyl sulfosuccinate—70% active

| Example Compositions:                                                  |                          |              |                          |              |
|------------------------------------------------------------------------|--------------------------|--------------|--------------------------|--------------|
|                                                                        | Compo-<br>sition<br>1, % | Solids,<br>% | Compo-<br>sition<br>2, % | Solids,<br>% |
| Intratex N*<br>(s.a.c.)                                                | —                        | —            | 18.9                     | 3.8          |
| Intratex N-1*                                                          | 25                       | 5            | —                        | —            |
| Ammonium Thiocyanate                                                   | 6.00                     | 6            | —                        | —            |
| Citric Acid<br>(50% solution)                                          | 14.30                    | 7.15         | —                        | —            |
| Sulfuric Acid                                                          | —                        | —            | 1.11                     | 1.1          |
| Tamol SN (sodium<br>salt of condensed<br>naphthalene<br>sulfonic acid) | 4.00                     | 3.9          | 7.32                     | 7.1          |
| Monawet MB-45<br>(di-isobutyl<br>sulfosuccinate)                       | 20.00                    | 9            | —                        | —            |
| Epsom Salt<br>(Magnesium Sulfate)                                      | 6.00                     | 6            | —                        | —            |
| Demineralized Water                                                    | 24.7                     | 2.9          | —                        | —            |
|                                                                        | 33.03                    | 0            | 72.65                    | 0            |

\*Same concentration of same s.a.c., N-1 has pH 7, N has pH 10.5.

Any thiocyanate such as those listed in the Summary of the Invention is expected to be effective, although

\*Chemcogen DCG is sulfonated alkyl diphenylether—30-38% active.  
 \*Defoamer AC is a proprietary defoamer from Fuller Sales.  
 \*Sequestrene 30A is ethylene diamine tetraacetic acid.  
 \*<sup>1</sup>TM of Crompton & Knowles  
 \*<sup>2</sup>TM of Ciba Geigy  
 \*<sup>3</sup>TM of Mobay  
 \*<sup>4</sup>TM of Lyndal Chem.  
 \*\*grams per liter

The following tables provide other operating conditions and results, using the above dyebaths and the shown aftertreatments. Trials 3 and 4 were omitted because they had a slightly different, nonpreferred, formulation.

TABLE III

| Trial<br>I.D. | STAINING DATA                                    |                                              |                                              |
|---------------|--------------------------------------------------|----------------------------------------------|----------------------------------------------|
|               | Nominal Comp. 1<br>Add-on from<br>Dyebath, % owf | Nominal Comp. 1<br>Add-on from<br>A/T, % owf | Total<br>Nominal<br>Comp. 1<br>Add-on, % owf |
| 1             | 0                                                | 0                                            | 0                                            |
| 5             | 0                                                | 0                                            | 11.0                                         |
| 9             | 4.0                                              | 7.0                                          | 11.0                                         |
| 10            | 4.0                                              | 11.0                                         | 15.0                                         |
| 2             | 0                                                | 0                                            | 0                                            |
| 6             | 0                                                | 10.9                                         | 10.9                                         |
| 8             | 4.0                                              | 7.0                                          | 11.0                                         |
| 7             | 0                                                | 14.9                                         | 14.9                                         |
| 11            | 4.0                                              | 10.9                                         | 14.9                                         |
| 12            | 8.0                                              | 7.0                                          | 15.0                                         |
| 13            | 8.0                                              | 11.0                                         | 19.0                                         |

TABLE I

| Trial<br>I.D.* | Aftertreatment (A/T) Application Data               |                                              |                                           |                                                |                                                  |                |                                                |
|----------------|-----------------------------------------------------|----------------------------------------------|-------------------------------------------|------------------------------------------------|--------------------------------------------------|----------------|------------------------------------------------|
|                | Nominal<br>Comp. 1<br>Add-on from<br>Dyebath, % owf | Nominal<br>Comp. 1 Add-on<br>from A/T, % owf | Total Nominal<br>Comp. 1 Add-on,<br>% owf | Preheat<br>Liquor<br>Temperature,<br>°F. (°C.) | Carpet Tempera-<br>ture Before A/T,<br>°F. (°C.) | A/T<br>Liquor, | Post-A/T Car-<br>pet Temperature,<br>°F. (°C.) |
|                |                                                     |                                              |                                           | *F. (°C.)                                      | *F. (°C.)                                        | pH             | *F. (°C.)                                      |
| 1              | 0                                                   | 0                                            | 0                                         | 142 (61.1)                                     | 128 (53.3)                                       | 7.6            | 157-159 (69.4-70.6)                            |
| 5              | 0                                                   | 11.0                                         | 11.0                                      | 140 (60.0)                                     | 127-129 (52.8-53.9)                              | 2.9            | 155-156 (68.3-68.9)                            |
| 9              | 4.0                                                 | 7.0                                          | 11.0                                      | 141 (60.6)                                     | 129-130 (53.9-54.4)                              | 3.0            | 158-159 (70.0-70.6)                            |
| 10             | 4.0                                                 | 11.0                                         | 15.0                                      | 140 (60.0)                                     | 128-129 (53.3-53.9)                              | 2.9            | 155-157 (68.3-69.4)                            |
| 2              | 0                                                   | 0                                            | 0                                         | 142 (61.1)                                     | 128 (53.3)                                       | 7.6            | 156-158 (68.9-70.0)                            |
| 6              | 0                                                   | 10.9                                         | 10.9                                      | 140 (60.0)                                     | 127-129 (52.8-53.9)                              | 2.9            | 158-160 (70.0-71.1)                            |
| 8              | 4.0                                                 | 7.0                                          | 11.0                                      | 141 (60.6)                                     | 128-131 (53.3-55.0)                              | 3.0            | 158-159 (70.0-70.6)                            |
| 7              | 0                                                   | 14.9                                         | 14.9                                      | 140 (60.0)                                     | 128-129 (53.3-53.9)                              | 2.8            | 160-162 (71.1-72.2)                            |
| 11             | 4.0                                                 | 10.9                                         | 14.9                                      | 140 (60.0)                                     | 129-131 (53.9-55.0)                              | 2.9            | 157-158 (69.4-70.0)                            |
| 12             | 8.0                                                 | 7.0                                          | 15.0                                      | 140 (60.0)                                     | 129-130 (53.9-54.4)                              | 3.0            | 160-161 (71.1-71.7)                            |
| 13             | 8.0                                                 | 11.0                                         | 19.0                                      | 140 (60.0)                                     | 130 (54.4)                                       | 2.9            | 157-159 (69.4-70.6)                            |

\*Numbers 1, 5, 9 and 10 trials are normal carpet fabric; remaining numbers are high ICP carpet fabric. Trials 1 and 2 are controls.

Both fabrics are 40 oz/sq yd cut piles.

A/T Liquor Temperature ranged from 180-182° F. (82.2-83.3° C.).

8                   4.0                   7.0                   11.0

TABLE II

| Trial<br>I.D. | SOLUTION AND CARPET ANALYSIS DATA       |                                             |                                           |       |                                    |                          |                                           |                                     |
|---------------|-----------------------------------------|---------------------------------------------|-------------------------------------------|-------|------------------------------------|--------------------------|-------------------------------------------|-------------------------------------|
|               | Concurrent Portion (in Dyebath)         |                                             |                                           |       | Aftertreatment Portion             |                          |                                           |                                     |
|               | Target Nominal Comp. 1<br>Add-on, % owf | Nominal Comp. 1<br>Conc. in<br>Dyebath, g/l | Anal. Comp. 1<br>Conc. in<br>Dyebath, g/l | Calc. | Target<br>Nominal<br>Add-on, % owf | Conc.<br>Deliv.,<br>GPM* | Actual A/T<br>Spray Header<br>Pres., psig | Total A/T<br>Liquor<br>Deliv., GPM* |
| 1             | 0                                       | 0                                           | 0                                         | 0     | 0                                  | 0                        | 6.7                                       | 77                                  |
| 2             | 0                                       | 0                                           | 0                                         | 0     | 0                                  | 0                        | 6.6                                       | 76                                  |
| 5             | 0                                       | 0                                           | 0                                         | 0     | 11.2                               | 1.19                     | 6.5                                       | 75                                  |
| 6             | 0                                       | 0                                           | 0                                         | 0     | 11.2                               | 1.19                     | 6.6                                       | 76                                  |
| 7             | 0                                       | 0                                           | 0                                         | 0     | 15.2                               | 1.62                     | 6.6                                       | 76                                  |
| 8             | 4.0                                     | 10.0                                        | 9.2                                       | 3.7   | 7.2                                | 0.76                     | 6.6                                       | 76                                  |
| 9             | 4.0                                     | 10.0                                        | 9.2                                       | 3.7   | 7.2                                | 0.76                     | 6.6                                       | 76                                  |
| 10            | 4.0                                     | 10.0                                        | 9.2                                       | 3.7   | 11.2                               | 1.19                     | 6.7                                       | 77                                  |
| 11            | 4.0                                     | 10.0                                        | 9.3                                       | 3.7   | 11.2                               | 1.19                     | 6.7                                       | 76                                  |
| 12            | 8.0                                     | 20.0                                        | 16.8                                      | 6.7   | 7.2                                | 0.76                     | 6.6                                       | 76                                  |
| 13            | 8.0                                     | 20.0                                        | 16.8                                      | 6.7   | 11.2                               | 1.19                     | 6.5                                       | 75                                  |

Aftertreatment Portion

| Trial<br>I.D. | Aftertreatment Portion                       |                                   |                                             |                                                      | Concurrent and Aftertreatment Portion |                                                   |                                                    |                                                     |
|---------------|----------------------------------------------|-----------------------------------|---------------------------------------------|------------------------------------------------------|---------------------------------------|---------------------------------------------------|----------------------------------------------------|-----------------------------------------------------|
|               | Calc.<br>Nominal<br>A/T Liquor<br>Conc., g/l | Anal. A/T<br>Liquor<br>Conc., g/l | Comp. 1<br>Add-on<br>from Set-<br>up, % owf | Calc. Comp.<br>1 Add-on<br>from Ana-<br>lysis, % owf | Target<br>Comp. 1<br>Add-on,<br>% owf | Calc. Comp.<br>1 Add-on<br>from Set-<br>up, % owf | Calc. Comp. 1<br>Add-on from<br>ANALYSIS,<br>% owf | Anal. Comp.<br>1 Add-on<br>from Car-<br>pets, % owf |
| 1             | 0                                            | 0                                 | 0                                           | 0                                                    | 0                                     | 0                                                 | 0                                                  | 0                                                   |
| 2             | 0                                            | 0                                 | 0                                           | 0                                                    | 0                                     | 0                                                 | 0                                                  | 0                                                   |
| 5             | 17.4                                         | 14.8                              | 11.0                                        | 9.3                                                  | 11.2                                  | 11.0                                              | 9.3                                                | 10.6                                                |
| 6             | 17.2                                         | 14.8                              | 10.9                                        | 9.4                                                  | 11.2                                  | 10.9                                              | 9.4                                                | 10.9                                                |
| 7             | 23.3                                         | 22.4                              | 14.9                                        | 14.3                                                 | 15.2                                  | 14.9                                              | 14.3                                               | 16.3                                                |
| 8             | 11.0                                         | 11.6                              | 7.0                                         | 7.4                                                  | 11.2                                  | 11.0                                              | 11.1                                               | 10.7                                                |
| 9             | 11.0                                         | 11.6                              | 7.0                                         | 7.4                                                  | 11.2                                  | 11.0                                              | 11.1                                               | 11.1                                                |
| 10            | 17.0                                         | 18.4                              | 11.0                                        | 11.9                                                 | 15.2                                  | 15.0                                              | 15.6                                               | 14.0                                                |
| 11            | 17.2                                         | 18.4                              | 10.9                                        | 11.7                                                 | 15.2                                  | 14.9                                              | 15.4                                               | 15.4                                                |
| 12            | 11.0                                         | 11.2                              | 7.0                                         | 7.1                                                  | 15.2                                  | 15.0                                              | 13.8                                               | 15.8                                                |
| 13            | 17.4                                         | 13.6                              | 11.0                                        | 8.6                                                  | 19.2                                  | 19.0                                              | 15.3                                               | 19.6                                                |

Line speed for both fabric was 30 ft/min.

Throughput = 99.8 lb carpet/min.

Actual dyeing wet pick-up was 400% in all cases.

Aftertreatment wet pick-up was always between 626 and 643%.

Aftertreatment pH was always between 2.8 and 3.0 except control was 7.6.

\*gallons per minute

TABLE III-continued

| STAINING DATA |     |      |      |  |  |  |
|---------------|-----|------|------|--|--|--|
| 7             | 0   | 14.9 | 14.9 |  |  |  |
| 11            | 4.0 | 10.9 | 14.9 |  |  |  |
| 12            | 8.0 | 7.0  | 15.0 |  |  |  |
| 13            | 8.0 | 11.0 | 19.0 |  |  |  |

Stain Rating<sup>1</sup> (0 = best 10 = worst)  
Time Before Blotting with Water, Hours

| Trial I.D. | 1    | 4    | 7    | 24   | 4         | 24          |
|------------|------|------|------|------|-----------|-------------|
|            |      |      |      |      | Originals | After s.c.* |
| 1          | 8.5  | 8.5  | 8.5  | 8.5  | 8.5       | 8.5         |
| 5          | 0.25 | 0.25 | 0.25 | 0.25 | 4.5       | 5.0         |
| 9          | 0    | 0    | 0    | 0    | 3.5       | 4.5         |
| 10         | 0    | 0    | 0    | 0    | 3.0       | 4.0         |
| 2          | 9.0  | 9.0  | 9.0  | 9.0  | 8.0       | 8.5         |
| 6          | 2.5  | 2.5  | 2.5  | 2.5  | 4.5       | 5.5         |
| 8          | 0.1  | 0.5  | 0.1  | 0.25 | 2.5       | 4.0         |
| 7          | 0.25 | 1.5  | 1.5  | 1.5  | 5.0       | 6.0         |
| 11         | 0    | 0.1  | 0.1  | 0.25 | 3.0       | 4.0         |
| 12         | 0    | 0    | 0    | 0.1  | 1.0       | 2.0         |
| 13         | 0    | 0    | 0    | 0    | 1.0       | 1.0         |

\*steam cleaning

2 passes of detergent solution using conventional steam cleaning equipment. Detergent solution: 1 oz./gal. ALL-IN-ONE (Certified Chemical & Equipment, Cleveland, OH).

<sup>1</sup>See Example 6, Part 2, "Performance", "Drop Test".

TABLE IV

| REPELLENCY AND COLORFASTNESS DATA |                      |                     |                     |                     |                             |                               |
|-----------------------------------|----------------------|---------------------|---------------------|---------------------|-----------------------------|-------------------------------|
| Trial I.D.                        | from Dye-bath, % owf | Comp. 1 Add-on from | Comp. 1 Add-on from | Total Nominal Comp. |                             |                               |
|                                   |                      |                     |                     | 1. Add-on, % owf    | Repellency <sup>3</sup> Oil | Repellency <sup>3</sup> Water |
| 1                                 | 0                    | 0                   | 0                   | 0                   | 5.0                         | 4.0                           |
| 5                                 | 0                    | 11.0                | 11.0                | 5.0                 | 4.0                         |                               |
| 9                                 | 4.0                  | 7.0                 | 11.0                | 4.0                 | 4.0                         |                               |
| 10                                | 4.0                  | 11.0                | 15.0                | 4.5                 | 3.5                         |                               |
| 2                                 | 0                    | 0                   | 0                   | 5.0                 | 5.0                         |                               |
| 6                                 | 0                    | 10.9                | 10.9                | 5.0                 | 4.0                         |                               |
| 8                                 | 4.0                  | 7.0                 | 11.0                | 5.0                 | 5.0                         |                               |
| 7                                 | 0                    | 14.9                | 14.9                | 5.0                 | 4.0                         |                               |
| 11                                | 4.0                  | 10.9                | 14.9                | 4.0                 | 4.0                         |                               |

20

TABLE IV-continued

| REPELLENCY AND COLORFASTNESS DATA |    |     |      |     |     |     |
|-----------------------------------|----|-----|------|-----|-----|-----|
| 5                                 | 6  | 4.0 | 4.0  | 3.0 | 2.5 | 2.5 |
|                                   | 8  | 4.5 | 4.0  | 3.5 | 3.0 | 2.5 |
|                                   | 7  | 4.0 | 4.0  | 3.0 | 3.0 | 2.5 |
|                                   | 11 | 4.0 | 3.75 | 3.5 | 3.0 | 3.0 |
|                                   | 12 | 4.0 | 3.25 | 3.0 | 3.0 | 2.5 |
|                                   | 13 | 3.5 | 3.0  | 3.0 | 2.5 | 2.5 |

\*AATCC 16E fading unit

\*\*cycles

<sup>1</sup>AATCC 129

<sup>2</sup>AATCC 164

<sup>3</sup>Oil Repellency

AATCC TM-118, Oil Repellency: Hydrocarbon Resistance Test.

Water Repellency

DuPont Isopropanol/water series

1. 2/98 IPA/Water (55)

2. 5/95 IPA/Water (47)

3. 10/90 IPA/Water (40)

4. 20/80 IPA/Water (33)

5. 30/70 IPA/Water (28)

Numbers in parentheses represents surface tension of the test fluids.

10

TABLE V

| BENZOYL PEROXIDE SPOTTING DATA* |                |             |             |         |                 |                                            |
|---------------------------------|----------------|-------------|-------------|---------|-----------------|--------------------------------------------|
| Trial I.D.                      | Dyebath, % owf | Comp. 1     | Comp. 1     | Total   | Spot Visibility |                                            |
|                                 |                | Add-on from | Add-on from | Nominal | Agent           | Benzoyl Peroxide Conc., % Soln. in Acetone |
| 1                               | 0              | 0           | 0           | 0       | 6.5             | 7.0                                        |
| 5                               | 0              | 11.0        | 11.0        | 0       | 1.0             | 2.0                                        |
| 9                               | 4.0            | 7.0         | 11.0        | 0       | 1.0             | 2.0                                        |
| 10                              | 4.0            | 11.0        | 15.0        | 0       | 2.0             | 2.0                                        |
| 2                               | 0              | 0           | 0           | 5.0     | 6.5             | 6.5                                        |
| 6                               | 0              | 10.9        | 10.9        | 0       | 1.0             | 1.5                                        |
| 8                               | 4.0            | 7.0         | 11.0        | 0       | 1.0             | 2.0                                        |
| 7                               | 0              | 14.9        | 14.9        | 0       | 0.5             | 1.0                                        |
| 11                              | 4.0            | 10.9        | 14.9        | 0       | 1.0             | 2.0                                        |
| 12                              | 8.0            | 7.0         | 15.0        | 0       | 0.5             | 1.5                                        |
| 35                              | 13             | 8.0         | 11.0        | 19.0    | 0               | 0.5                                        |

\*Sample spotted with 1-ml of benzoyl peroxide solution and exposed in chamber at 90° F. (32.2° C.) and 80% R.H. for three days (color change ceases).

TABLE VI

| SOILING DATA |                |             |             |                       |               |        |       |
|--------------|----------------|-------------|-------------|-----------------------|---------------|--------|-------|
| Trial I.D.   | Dyebath, % owf | Comp. 1     | Comp. 1     | Total Nominal Comp. 1 | Treads        |        | Total |
|              |                | Add-on from | Add-on from | Add-on, % owf         | Accl.* Method | JTCC** | Soil  |
| 1            | 0              | 0           | 0           | 0                     | 5.0           | 5.5    | 7.0   |
| 4            | 0              | 10.9        | 10.9        | 5.5                   | 6.0           | 7.0    | 18.5  |
| 5            | 0              | 11.0        | 11.0        | 5.5                   | 6.0           | 7.5    | 19.0  |
| 9            | 4.0            | 7.0         | 11.0        | 4.5                   | 6.0           | 7.5    | 18.0  |
| 10           | 4.0            | 11.0        | 15.0        | 4.5                   | 6.0           | 7.5    | 18.0  |
| 2            | 0              | 0           | 0           | 5.5                   | 4.0           | 5.5    | 15.0  |
| 3            | 0              | 10.9        | 10.9        | 5.5                   | 4.5           | 6.0    | 16.0  |
| 6            | 0              | 10.9        | 10.9        | 5.5                   | 5.5           | 6.5    | 17.5  |
| 8            | 4.0            | 7.0         | 11.0        | 4.0                   | 5.0           | 7.0    | 16.0  |
| 7            | 0              | 14.9        | 14.9        | 5.5                   | 5.5           | 7.0    | 18.0  |
| 11           | 4.0            | 10.9        | 14.9        | 4.0                   | 4.5           | 7.0    | 15.5  |
| 12           | 8.0            | 7.0         | 15.0        | 4.5                   | 5.5           | 7.0    | 17.0  |
| 13           | 8.0            | 11.0        | 19.0        | 4.5                   | 5.5           | 7.0    | 17.0  |

\*Accelerated soiling conducted at Petersburg Rehabilitation Center using "natural soil" with 2.5% mineral oil added.

\*\*John Tyler Community College Maintenance Hall.

| Trial I.D. | Grey Scale Rating |                            |                                       |        |      |
|------------|-------------------|----------------------------|---------------------------------------|--------|------|
|            | Lightfastness     | Ozonefastness <sup>1</sup> | NO <sub>2</sub> <sup>2</sup> Fastness | 1 cy** | 3 cy |
| 12         | 8.0               | 7.0                        | 15.0                                  | 4.0    | 4.0  |
| 13         | 8.0               | 11.0                       | 19.0                                  | 4.0    | 3.5  |

60

### Example 1—Conclusions

The two-step process with composition gives considerably better stain resistance than the aftertreatment (only) process, at equal total add-on levels. This shows potential for achieving acceptable performance at lower total add-on levels.

The two-step process also gives acceptable stain resistance on the "high ICP" substrate at levels comparable

to that currently being used for s.a.c. normal substrates by aftertreatment only.

Stain resistance improves and lightfastness is adversely effected (yellowing) as the Composition 1 concentration in the concurrent portion increases, with total add-on level constant. Acceptable yellowing and stain resistance was achieved at 4% on the weight of the fiber of Composition 1 in the concurrent portion.

"Optimum" two-step systems had improved ozone and benzoyl peroxide (B.P.) spotting resistance properties. Some reduction does occur as the concentration applied by the aftertreatment portion is reduced in favor of the concurrent portion.

#### Example 1—Summary of Results

##### Staining Performance Table III

In general, the standard Superba heat set (H/S) substrate performed better than the high ICP substrate at equivalent application conditions, while analyzed add-ons were equal. This is normally observed because of undesired deep penetration of s.a.c. into fiber of high ICP.

When applied by aftertreatment only, Composition 1 on the high ICP fabric did not yield acceptable staining performance. When the level of Composition 1 was increased from 11 to 15% owf on the high ICP fabric, stain resistance was further improved to a "Marginal" performance level (stain rating of 1.5 at 4- and 24-hour blot times).

The two-step process gave considerably better stain resistance than the aftertreatment only process on both substrates, at equal total application levels. No staining at 24 hours was obtained on the Superba H/S fabric using 4% on the weight of the fiber in the Dyebath and 7% on the weight of the fiber in the A/T. These same levels on the high ICP substrate gave staining performance equal to the Superba fabric aftertreated (only) with 11% on the weight of the fiber of Composition 1 (stain rating of 0.5 at 24 hours).

#### Example 1—Summary of Results

##### Colorfastness Table IV

No light induced yellowing was observed at 20 AFU on any of the trials conducted, but begin to be noticed at 40 AFU.

Light induced yellowing (at 40 AFU) became more noticeable as the amount in the concurrent portion was increased (and aftertreatment was reduced). Trials with 8% on the weight of the fiber Composition 1 in the concurrent portion (high ICP substrate) were marginal to unacceptable for lightfastness.

The improvement in resistance to ozone fading, obtained with Composition 1 by aftertreatment was also observed with Composition 1 and also using the two-step process with Composition 1 (at lower level).

##### Benzoyl Peroxide Spotting Table V

The two-step process gave only a slight reduction in the benzoyl peroxide spotting performance than the aftertreatment process, at equal add-on levels.

##### Repellency Table IV

There was no significant effect in any of the trials on oil and water repellency. As the amount of Composition 1 (and magnesium sulfate) in the concurrent portion was increased, the oil repellency tended to decrease slightly.

##### Soiling Table VI

Only a slight negative effect in soiling was observed on all trial samples compared to the control.

Composition 1 showed slightly more soiling when applied by aftertreatment, as the concentration applied was increased.

With total add-on constant, the two-step process had less impact on soiling than aftertreatment alone.

#### Two-Step Process Guidelines (Best Mode) For The Continuous Application of Composition 1

##### Concurrent (with dyestuffs) Portion:

For Suessen H/S Substrates: 2.0% owf  
For Superba H/S Substrates: 3.0% owf  
For "High ICP" Substrates: 4.0-5.0% owf

##### Dyebath Make-up Procedure

1st—Wetting and leveling agents (defoamer, if required)

2nd—Composition and Epsom Salt\*\* (MgSO<sub>4</sub>—7H<sub>2</sub>O) (0.5% owf Epsom Salt for each 4.0% owf Composition 1)

3rd—0.25-0.50 g/l Sequestering agent (EDTA)

4th—Dyestuffs

5th—Adjust to desired pH with either acetic acid, ammonia or caustic soda\*

##### Notes:

\*Composition 1 has low pH. Use in the dyebath will result in pH's of 3.0-3.5, requiring an alkali to adjust pH.

\*\*Only phosphates which form water-soluble complexes with magnesium ion may be used in the presence of magnesium sulfate.

##### Aftertreatment Portion

##### Composition 1 Concentration:

For Suessen H/S Substrates: 3.0% owf  
For Superba H/S Substrates: 5.0% owf  
For "High ICP" Substrates: 7.0-8.0%

##### Application Parameters

45 Preheat/wash spray at 160° F. (71.1° C.) and extract (vacuum) to 75-125% w.p.u. to give carpet temperature of 140° F. (60° C.).

46 Apply treatment solution at 180° F. (81.2° C.) and 400-500% w.p.u. to give a post-A/T carpet temperature of 160° F. (71.1° C.).

##### Example 2

55 This is a further example of the continuous aftertreatment process of the invention, using Composition 2 in the treatment of the carpet fabric. The fabrics treated were (a) a fabric tufted from an 1186 denier continuous filament textured medium dye fiber in a Superba heatset (H/S) yarn to a 28-ounce cut pile fabric and (b) a textured 3.15/2 cotton count yarn from a 19 denier per filament staple deep dye fiber heat in a Suessen and tufted into 48-ounce fabric. Both were pretreated with the fluorocarbon of Example 1 and were to be dyed light gray. The nominal application conditions were 140° F. (60° C.) preheat water temperature, 180° F. (81.2° C.) application liquor temperature, 500 to 600% w.p.u. application liquor, the dyes and dyebath additives were as in Example 1, except no sequestrene was used. No Composition 2 or other s.a.c. was added to the

dyebath. The following Tables show the application conditions and results.

TABLE XI-continued

TABLE VII

| APPLICATION DATA |                            |                                    |                                         |                                     |                        |                              |
|------------------|----------------------------|------------------------------------|-----------------------------------------|-------------------------------------|------------------------|------------------------------|
| Trial I.D.       | Nominal Comp. 2 Applied, % | Target Nominal s.a.c. Level, % owf | Target Nominal Epsom Salts Level, % owf | Actual A/T Spray Header Pres., psig | A/T Liquor Deliv., GPM | Target A/T Liquor Conc., g/l |
| 1                | 0                          | 0                                  | 0                                       | 6.2                                 | 73.3                   | 0                            |
| 2                | 15.0                       | 2.8                                | 0                                       | 6.2                                 | 73.3                   | 25.0                         |
| 3                | 0                          | 0                                  | 0                                       | 6.5                                 | 75.2                   | 0                            |
| 4                | 9.0                        | 1.7                                | 0                                       | 6.5                                 | 75.2                   | 17.2                         |

Actual w.p.u. was between 523 and 532%, pH was 8.3 for control; 3.0 for Trial 2; 3.3 for Trial 4. Preheat liquor temperature was 140° F. (60° C.). Carpet temperature was 127-130° F. (52.8-54.4° C.). Application liquor temperature was 179-182° F. (81.7-83.5° C.) and carpet temperature was 156-161° F. (68.9-71.7° C.).

| Trial I.D. | Calc. Conc. Comp. 2 Liquor g/l | Anal. Conc. Comp. 2 Liquor g/l | Calc. Comp. 2 Add-on from Set-up % owf | Calc. s.a.c. on from Anal. A/T Liquor % owf | Calc. s.a.c. Add-on from Carpets % owf | Calc. Epsom Salt Add-on % owf |
|------------|--------------------------------|--------------------------------|----------------------------------------|---------------------------------------------|----------------------------------------|-------------------------------|
| 1          | 0                              | 0                              | 0                                      | 0                                           | 0                                      | 0                             |
| 2          | 30.4                           | 21.2                           | 17.7                                   | 3.4                                         | 2.3                                    | 2.62                          |
| 3          | 0                              | 0                              | 0                                      | 0                                           | 0                                      | 0                             |
| 4          | 20.9                           | 14.4                           | 10.9                                   | 2.1                                         | 1.5                                    | 1.89                          |

Actual w.p.u. was between 523 and 532%, pH was 8.3 for control; 3.0 for Trial 2; 3.3 for Trial 4. Preheat liquor temperature was 140° F. (60° C.). Carpet temperature was 127-130° F. (52.8-54.4° C.). Application liquor temperature was 179-182° F. (81.7-83.5° C.) and carpet temperature was 156-161° F. (68.9-71.7° C.).

TABLE VIII

STAINING PERFORMANCE, DURABILITY TO  
STEAM CLEANING AND CHANGE-OF-SHADE DATA

| Sample I.D. | Nominal Comp. 2 Applied, % | Stain Rating (0 = best, 10 = worst) |      |      |     |      |     | S.C.** | Shade Change* |
|-------------|----------------------------|-------------------------------------|------|------|-----|------|-----|--------|---------------|
|             |                            | 0.05                                | 0.5  | 1    | 4   | 8    | 24  |        |               |
| 1           | 0                          | 8.5                                 | 8.5  | 8.5  | 8.5 | 8.5  | 7.0 | —      |               |
| 2           | 15                         | 0.25                                | 0.25 | 0.75 | 1.5 | 1.75 | 2.0 | 5.0    | M-N (Y)       |
| 3           | 0                          | 4.5                                 | 7.0  | 7.0  | 7.0 | 7.0  | 7.0 | 7.0    | —             |
| 4           | 9                          | 0                                   | 0    | 0    | 0.1 | 0.1  | 0.1 | 3.0    | M (Y)         |

\*N = no, acceptable; M = marginal; Y = yellow. Letter in parentheses indicates direction of color change from the control.

\*\*steam cleaned.

TABLE IX

| Sample I.D. | Nominal Comp. 2 Applied, % | COLORFASTNESS DATA |     |     |     |     |                            |     |      |  |  |
|-------------|----------------------------|--------------------|-----|-----|-----|-----|----------------------------|-----|------|--|--|
|             |                            | Grey Scale Rating  |     |     |     |     | NO <sub>2</sub> * Fastness |     |      |  |  |
|             |                            | Lightfastness, AFU | 20  | 40  | 1   | 2   | 3                          | 5   | 1 cy |  |  |
| 1           | 0                          | 4.0                | 3.0 | 3.0 | 2.5 | 2.0 | 1.0                        | 2.5 |      |  |  |
| 2           | 15.0                       | 2.5                | 3.0 | 3.0 | 2.5 | 2.5 | 2.0                        | 1.0 |      |  |  |
| 3           | 0                          | 4.5                | 3.5 | 3.5 | 3.0 | 2.5 | 2.0                        | 2.5 |      |  |  |
| 4           | 9.0                        | 3.5                | 3.5 | 3.5 | 3.0 | 3.0 | 2.5                        | 1.5 |      |  |  |

\*High R.H. nitrogen dioxide (AATCC TM-164).

TABLE X

BENZOYL PEROXIDE SPOTTING DATA\*

| Sample I.D. | Nominal Comp. 2 Applied, % | Spot Visibility (0 = Invisible; 10 = Bright) Originals |      |      |     |     |      |      |      |     |     |
|-------------|----------------------------|--------------------------------------------------------|------|------|-----|-----|------|------|------|-----|-----|
|             |                            | Benzoyl Peroxide Conc., % Solution in Acetone          |      |      |     |     |      |      |      |     |     |
|             |                            | 0.01                                                   | 0.05 | 0.10 | 1.0 | 5.0 | 0.01 | 0.05 | 0.10 | 1.0 |     |
| 1           | 0                          | 2.0                                                    | 7.5  | 8.0  | 9.0 | 9.5 | 1.0  | 5.0  | 7.0  | 9.0 | 9.5 |
| 2           | 15                         | 1.0                                                    | 6.5  | 7.0  | 8.5 | 8.5 | 0.25 | 5.0  | 7.0  | 8.5 | 9.0 |
| 3           | 0                          | 2.0                                                    | 7.5  | 8.0  | 9.0 | 9.5 | 0.5  | 5.0  | 7.0  | 8.5 | 9.0 |
| 4           | 9                          | 2.0                                                    | 7.5  | 8.0  | 8.5 | 8.5 | 0.3  | 4.5  | 6.5  | 8.0 | 9.0 |

\*Sample spotted with 1 ml of benzoyl peroxide solution and exposed in chamber at 90° F. (32.2° C.) and 80% R.H. for three days (color change ceases).

TABLE XI

| Sample I.D. | Nominal Comp. 2 Applied, % | REPELLENCY DATA (FINISHED CARPETS) |       |
|-------------|----------------------------|------------------------------------|-------|
|             |                            | Oil                                | Water |
| 1           | 0                          | 4.0                                | 4.0   |

REPELLENCY DATA (FINISHED CARPETS)

| Sample I.D. | Nominal Comp. 2 Applied, % | REPELLENCY DATA (FINISHED CARPETS) |       |
|-------------|----------------------------|------------------------------------|-------|
|             |                            | Oil                                | Water |
| 2           | 15.0                       | 4.0                                | 4.5   |
| 3           | 0                          | 3.0                                | 4.0   |

TABLE XI-continued

| REPELLENCY DATA (FINISHED CARPETS) |                 |            |       |
|------------------------------------|-----------------|------------|-------|
| Sample                             | Nominal Comp. 2 | Repellency |       |
| I.D.                               | Applied, %      | Oil        | Water |
| 4                                  | 9.0             | 3.0        | 4.5   |

This Example 2 demonstrates the effectiveness of the sulfonated aromatic condensate with only a dispersing agent and further demonstrates the effectiveness of the continuous aftertreatment process of this invention.

## EXAMPLE 3

## Part 1

This example demonstrates the effective use of the process of this invention on fabric which has not been previously treated with any fluorocarbon compound for antisoiling properties. The Composition 2 used in the continuous aftertreatment process (no two step) of this invention as set forth in Example 1. Dyebath formulation was as in Example 2. Conditions were as in Example 1, more specifically, preheat water temperature was 195° F. (90.6° C.) at 100% w.p.u. to achieve carpet temperature of 135°-140° F. (57.2° to 60° C.). After-treatment liquor temperature was 180°-185° F. (82.2° to 85° C.) to achieve carpet temperature of 160°-170° F. (71.1° to 76.7° C.). Aftertreatment dwell time was 30 seconds before washing at 40:1 liquor to fabric ratio, hydroextraction and drying. Both compositions were applied at both 1.5 and 3.0% on the weight of the fabric. Samples of fabric pretreated with fluorocarbons, which are also part of the invention, were run alongside the fabric untreated with fluorocarbon. The results show that higher amounts of sulfonated aromatic condensate must be applied to the fabric untreated with fluorocarbon to achieve the nearly same level of stain resistance. The following tables give application conditions and results.

TABLE XII

| EVALUATION OF STAIN BLOCKING FOR CONTINUOUS AFTERTREATMENT |                    |                                 |                        |                          |                        |                                   |                        |                     |                        |
|------------------------------------------------------------|--------------------|---------------------------------|------------------------|--------------------------|------------------------|-----------------------------------|------------------------|---------------------|------------------------|
| Sample                                                     | Nominal Add-on, %* | Stain Rating Total <sup>1</sup> |                        | 20 AFU Rank <sup>2</sup> |                        | NO <sub>2</sub> Rank <sup>2</sup> |                        | Soiling Rating**    |                        |
|                                                            |                    | Fabric With Fluoro.             | Fabric Without Fluoro. | Fabric With Fluoro.      | Fabric Without Fluoro. | Fabric With Fluoro.               | Fabric Without Fluoro. | Fabric With Fluoro. | Fabric Without Fluoro. |
| 1                                                          | 0                  | 54.0                            | 45.0                   | 2                        | 3                      | 1                                 | 1                      | 4                   | 8                      |
| 2                                                          | 3.0                | 1.5                             | 1.4                    | 4                        | 7                      | 2                                 | 2                      | 9.5                 | 9                      |
| 3                                                          | 3.0                | 0.3                             | 0.3                    | 4                        | 9                      | 2                                 | 3                      | 10                  | 10                     |
| 4                                                          | 3.0                | 1.2                             | 1.5                    | 4                        | 9                      | 2                                 | 2                      | 5.5                 | 7.5                    |

\*Samples 2 and 4 applied at pH 3. Samples 1 and 3 were applied at pH 2.

<sup>1</sup>Total of ratings at 1, 4, 7 and 24-hour tests. High numbers indicate most stain.

<sup>2</sup>Lower numbers are better.

\*\*Soiling evaluated under Accelerated Method, 0 = best, 10 = worst.

| Sample I.D. | Nominal Add-on, % | S.a.c. Analyzed, % o/wf* |                        |
|-------------|-------------------|--------------------------|------------------------|
|             |                   | Fabric With Fluoro.      | Fabric Without Fluoro. |
| 1           | —                 | 0                        | 0                      |
| 2           | 3.0               | 3.09                     | 2.96                   |
| 3           | 3.0               | 3.47                     | 3.36                   |
| 4           | 3.0               | 2.94                     | 2.86                   |

Samples 2 and 4 were applied at pH 3. Samples 1 and 3 were applied at pH 2.

\*Extracted from carpets with 0.1N NaOH for four hours and analyzed by HPLC against original material.

## EXAMPLE 3

## Part 2

The conditions of Example 3—Part 1 were repeated except Composition 1 was used with the results shown in the following tables. All fabric was without fluorocarbon treatments.

TABLE XIV

| STAINING AND CHANGE-OF-SHADE DATA |        |                 |                                     |      |      |      |                      |              |  |
|-----------------------------------|--------|-----------------|-------------------------------------|------|------|------|----------------------|--------------|--|
| Trial                             | Add-on | Nominal Comp. 1 | Stain Rating (0 = best, 10 = worst) |      |      |      | Time Before Blotting |              |  |
|                                   |        |                 | With Water, Hr                      | 1    | 4    | 7    | 24                   | Shade Change |  |
| 15                                | 1      | —               | 7.0                                 | 7.0  | 7.0  | 7.0  | 7.0                  | —            |  |
|                                   | 2      | 5.0             | 0.25                                | 1.0  | 1.0  | 0.75 | 0.75                 | M (Y)        |  |
|                                   | 3      | 6.0             | 0.1                                 | 0.75 | 0.75 | 0.5  | 0.5                  | M (Y)        |  |
|                                   | 4      | 7.0             | 0.1                                 | 0.25 | 0.25 | 0.25 | 0.25                 | M (Y)        |  |
|                                   | 5      | 8.0             | 0.1                                 | 0.25 | 0.25 | 0.25 | 0.25                 | M (Y)        |  |

TABLE XV

| Trial | Add-on | Nominal Comp. 1 | COLORFASTNESS DATA |     |                   |     |     |
|-------|--------|-----------------|--------------------|-----|-------------------|-----|-----|
|       |        |                 | Grey Scale Rating  |     | Ozonefastness, cy |     |     |
|       |        |                 | Lightfastness, AFU | 20  | 40                | 1   | 3   |
| 25    |        |                 |                    |     |                   |     |     |
|       | 1      | —               | 4.0                | 3.5 | 3.5               | 2.0 | 3.0 |
|       | 2      | 5.0             | 4.5                | 4.0 | 4.0               | 3.0 | 2.5 |
|       | 3      | 6.0             | 4.5                | 4.0 | 4.0               | 3.5 | 2.5 |
|       | 4      | 7.0             | 4.5                | 4.0 | 4.0               | 3.5 | 2.5 |
|       | 5      | 8.0             | 4.5                | 4.0 | 4.5               | 4.0 | 2.5 |

TABLE XVI

| Trial | Add-on | Nominal Comp. 1 | ANALYSIS DATA |           |              |           |                      |
|-------|--------|-----------------|---------------|-----------|--------------|-----------|----------------------|
|       |        |                 | Nominal Conc. | Anal. A/T | Liquor Conc. | Anal. A/T | Anal. A/T from Rinse |
|       |        |                 |               |           |              |           | s.a.c.               |
| 35    |        |                 |               |           |              |           |                      |
|       | 1      | —               | —             | —         | —            | —         | N/D**                |
|       | 2      | 5.0             | 12.5          | 11.8      | 4.7          | 5.1       | N/D                  |
|       | 3      | 6.0             | 15.0          | 15.0      | 6.0          | 7.3       | N/D                  |
|       | 4      | 7.0             | 17.5          | 19.6      | 7.8          | 7.5       | N/D                  |
|       | 5      | 8.0             | 20.0          | 23.5      | 9.4          | 8.3       | N/D                  |

\*Applied at 400% w.p.u.

\*\*Non-detected

## EXAMPLE 4

The process and conditions of dyeing formulations of Example 2 using Composition 2 were repeated with and without citric acid to adjust pH in the continuous aftertreatment application process of this invention the fab-

ric was in 32 ounce per square yard cut pile construction of a 1185 denier bulked continuous filament, Superba H/S, beck-dyed grey. The fiber had been treated with fluorocarbon for antisoil properties. Also all dispersing agents (Tamol) were omitted from Composition 2 for another set of samples. Epsom salt (49% MgSO<sub>4</sub>) was added to another set of samples. Citric acid was used as a rinse and in the application liquor. Use of citric acid in the treatment liquor or to adjust pH resulted in improved yellowing of the sulfonated aromatic condensate treated fiber. The combination of Epsom salt and citric acid further reduced the tendency to yellow whether due to exposure to ozone or to NO<sub>2</sub>. The following tables provide application conditions and results.

5 10 15

TABLE XIX

EVALUATION OF CITRIC ACID - USE FOR CONCENTRATE pH ADJUSTMENT ON LIGHT INDUCED YELLOWING COLORFASTNESS DATA

| Sample I.D. | Grey Scale Rating  |                   |     |     |     |     | NO <sub>2</sub> * Fastness, 1 cy |
|-------------|--------------------|-------------------|-----|-----|-----|-----|----------------------------------|
|             | Lightfastness, AFU | Ozonefastness, cy | 1   | 2   | 3   | 5   |                                  |
| 6           | 4.0                | 3.5               | 3.0 | 2.5 | 1.5 | 1.0 | 2.5                              |
| 1           | 2.5                | 3.0               | 3.0 | 2.5 | 2.5 | 2.0 | 1.5                              |
| 2           | 2.5                | 3.0               | 3.0 | 2.5 | —   | —   | 1.5                              |
| 3           | 2.5                | 3.0               | 3.0 | 2.5 | —   | —   | 1.5                              |
| 4           | 3.0                | 3.0               | 3.5 | 3.0 | 3.0 | 2.5 | 1.5                              |
| 5           | 3.0                | 3.0               | 3.5 | 3.0 | —   | —   | 2.0                              |
| 7           | 2.5                | 3.0               | 3.0 | 3.0 | —   | —   | 1.5                              |
| 8           | 2.5                | 3.0               | 3.0 | 2.5 | —   | —   | 1.5                              |

TABLE XVII

EVALUATION OF CITRIC ACID - USE FOR CONCENTRATE pH ADJUSTMENT ON LIGHT INDUCED YELLOWING APPLICATION AND ANALYSIS DATA

| Sample I.D. | s.a.c. Used   | Nominal |                                              |                    | Appl. pH | Rinse                    | s.a.c. Analyzed % |
|-------------|---------------|---------|----------------------------------------------|--------------------|----------|--------------------------|-------------------|
|             |               | s.a.c.  | Applied %                                    | Other Agents/Conc. |          |                          |                   |
| 6           | Not Treated   | 0       | —                                            |                    | 7.5      | Normal - Cold Water      | 0                 |
| 1           | Composition 2 | 3.0     | —                                            |                    | 3.1      | Normal - Cold Water      | 1.87              |
| 2           | Composition 2 | 3.0     | —                                            |                    | 3.1      | 0.09 g/l Citric (pH 4.1) | 2.18              |
| 3           | Composition 2 | 3.0     | —                                            |                    | 3.1      | 0.25 g/l Citric (pH 3.5) | 2.29              |
| 4           | Composition 2 | 3.0     | —                                            |                    | 3.1      | 0.75 g/l Citric (pH 3.1) | 2.32              |
| 5           | Composition 2 | 3.0     | —                                            |                    | 3.1      | 5.9 g/l Citric (pH 2.5)  | 2.44              |
| 7           | Composition 2 | 3.0     | 0.09 g/l Citric Acid                         |                    | 3.1      | Normal - Cold Water      | 1.90              |
| 8           | Composition 2 | 3.0     | 0.09 g/l Citric Acid                         |                    | 3.1      | No Rinse                 | 2.10              |
| 9           | Composition 2 | 3.0     | 0.75 g/l Citric Acid                         |                    | 2.9      | Normal - Cold Water      | 2.04              |
| 10          | Composition 2 | 3.0     | 0.75 g/l Citric Acid                         |                    | 2.9      | No Rinse                 | 2.30              |
| 11          | Intratex N    | 3.0     | Citric Acid (pH adj)*                        |                    | 3.0      | Normal - Cold Water      | 2.67              |
| 12          | Intratex N    | 3.0     | Citric Acid (pH adj)*                        |                    | 3.0      | No Rinse                 | 2.39              |
| 13          | Intratex N    | 3.0     | 0.72% o/w Epsom Salt & Citric Acid (pH adj)* |                    | 3.0      | Normal - Cold Water      | 2.89              |
| 14          | Intratex N    | 3.0     | 0.72% o/w Epsom Salt & Citric Acid (pH adj)* |                    | 3.0      | No Rinse                 | 2.89              |

\*1.25 g/l citric acid required for pH adjustment.

Notes:

Carpet temperature before A/T ranged from 132 to 138° F. (55.6-58.9° C.).

A/T liquor temperature was 183 to 185° F. (83.9-85° C.).

Actual temperature after A/T ranged from 163 to 171° F. (72.8-77.2° C.).

|    |     |     |     |     |     |     |     |
|----|-----|-----|-----|-----|-----|-----|-----|
| 9  | 3.0 | 3.0 | 3.5 | 3.0 | 3.0 | 2.5 | 2.0 |
| 10 | 2.5 | 3.0 | 3.5 | 3.0 | 3.0 | 2.5 | 1.5 |
| 11 | 3.0 | 3.5 | 3.5 | 3.0 | —   | —   | 2.0 |
| 12 | 3.0 | 3.5 | 3.5 | 3.0 | —   | —   | 2.0 |
| 45 | 13  | 4.0 | 3.5 | 3.5 | 3.0 | 3.0 | 2.5 |
|    | 14  | 4.0 | 3.5 | 3.5 | 3.5 | 3.0 | 2.5 |

\*High R.H. nitrogen dioxide (AATCC TM-164).

TABLE XVIII

EVALUATION OF CITRIC ACID - USE FOR CONCENTRATE pH ADJUSTMENT ON LIGHT INDUCED YELLOWING STAINING PERFORMANCE AND CHANGE-OF-SHADE DATA

| Sample I.D. | Stain Rating (0 = best, 10 = worst) |      |      |      |      |      | Shade Change* |
|-------------|-------------------------------------|------|------|------|------|------|---------------|
|             | 0.05                                | 0.5  | 1    | 4    | 8    | 24   |               |
| 6           | 9.5                                 | 9.5  | 9.5  | 9.5  | 9.5  | 9.5  | —             |
| 1           | 0                                   | 0.25 | 0.5  | 1.0  | 1.0  | 1.0  | M-N           |
| 2           | 0                                   | 0.25 | 0.25 | 0.5  | 0.5  | 0.75 | M-N           |
| 3           | 0                                   | 0.25 | 0.25 | 0.5  | 0.75 | 1.0  | M-N           |
| 4           | 0                                   | 0.25 | 0.25 | 0.5  | 0.75 | 0.75 | M-N           |
| 5           | 0                                   | 0.25 | 0.5  | 0.5  | 1.0  | 1.5  | M-N           |
| 7           | 0                                   | 0.25 | 0.25 | 0.25 | 0.25 | 0.25 | M-N(Y)        |
| 8           | 0                                   | 0.25 | 0.25 | 0.5  | 1.0  | 1.0  | M-N(B)        |
| 9           | 0                                   | 0.25 | 0.25 | 0.25 | 0.5  | 0.75 | M-N(B)        |
| 10          | 0                                   | 0.1  | 0.1  | 0.5  | 0.5  | 0.5  | M-N           |
| 11          | 0.1                                 | 0.5  | 0.5  | 0.5  | 0.5  | 1.0  | M-N           |
| 12          | 0                                   | 0.25 | 1.0  | 2.0  | 2.5  | 2.5  | M-N           |
| 13          | 0                                   | 0.25 | 0.25 | 0.25 | 0.25 | 0.25 | M-N(B)        |
| 14          | 0                                   | 0.25 | 0.5  | 0.5  | 0.5  | 0.5  | M-N(B)        |

\*M = marginal, N = none, Y = yellow, B = blue

| Sample I.D. | BENZOYL PEROXIDE SPOTTING DATA*              |                                            |      |      |      | 5.0 |
|-------------|----------------------------------------------|--------------------------------------------|------|------|------|-----|
|             | Spot Visibility (0 = Invisible; 10 = Bright) | Benzoyl Peroxide Conc., % Soln. in Acetone | 0.01 | 0.05 | 0.10 | 1.0 |
| 6           | 3.0                                          | 7.0                                        | 8.0  | 9.0  | 9.5  |     |
| 1           | 0.75                                         | 5.5                                        | 6.5  | 7.5  | 8.0  |     |
| 13          | 0                                            | 0.25                                       | 0.5  | 1.5  | 2.5  |     |
| 14          | 0                                            | 0.25                                       | 0.5  | 1.5  | 2.5  |     |

\*Sample spotted with 1 ml of benzoyl peroxide solution and exposed in chamber at 90° F. (32.2° C.) and 80% R.H. for three days.

## EXAMPLE 5

The process on the fabric of Example 4 was repeated, also using Composition 2 with and without the Tamol dispersant, and also adding NH<sub>4</sub>SCN to show its benefits.

Following are the standard continuous process after-treatment conditions used:

Prewet/heat carpet at 195° F. (90.6° C.) and 100% w.p.u. to achieve a carpet temperature prior to treatment of 135° to 140° F. (57.2° to 60° C.).

Apply A/T liquor at 400% w.p.u. and 175° to 180° F. (79.4° to 82.2° C.) to achieve a post-A/T carpet temperature of 160° to 170° F. (71.1° to 76.7° C.).

Aftertreatment, 30-second dwell time before washing (at 40.1 liquor ratio), hydroextraction and drying.

### Summary of Results

#### 1. Application

The addition of NH<sub>4</sub>SCN to the Composition 2 bath was found to affect pH only at the lowest concentration. This is an indication of the buffering capacity of Composition 2 solutions.

During the make-up and running of the treatment solutions, it was observed that considerably more foaming occurs with Intratex-N alone than does Composition 2.

#### 2. Stain Resistance

Composition 2 tended to exhibit better staining performance than Intratex N alone at comparable levels. The differences between the two diminish as the overall concentration increases.

The addition of NH<sub>4</sub>SCN did not adversely affect the staining performance and, in fact, samples with NH<sub>4</sub>SCN tended to perform better than corresponding samples without NH<sub>4</sub>SCN. This difference diminishes as the Intratex N concentration increases and overall performance improves.

#### 3. Light and NO<sub>2</sub> Induced Yellowing (Table XXIII)

Intratex N and Tamol SN (by themselves) were found to behave differently when exposed to light. Intratex N yellows/browns severely at short light exposures (20 afu). This yellowing or browning then fades as the lightfastness exposure is continued. Tamol, on the other hand, greens when exposed to 20 afu and upon continued exposure the green fades to yellow. The overall rating of the shade change does not necessarily improve from the 20 to 40 afu exposures. The severity of shade change is about equal for Intratex N and Tamol SN.

The break of Composition 2 at short lightfastness exposures (20 afu) appears as a hybrid of Intratex N and Tamol SN alone (at the respective levels in Composition 2).

At both 20 and 40 afu, the break of Composition 2 samples were no worse-to-slightly better than the corresponding Intratex N and Tamol SN only samples.

The addition of NH<sub>4</sub>SCN gives a slight improvement in light induced yellowing. The reduction is greatest at the lower Intratex N levels and decreases as the Intratex N level increases. Similar behavior is observed between Composition 2 and Intratex N alone, but Tamol SN is less affected.

Yellowing diminishes as the NH<sub>4</sub>SCN level increases. The yellowing is significantly reduced using approximately 0.3% owf NH<sub>4</sub>SCN for every 1.0% owf Intratex N.

Tamol SN was found to be unaffected by exposure to NO<sub>2</sub>, while Composition 2 and Intratex N yellowed severely. The addition of NH<sub>4</sub>SCN improved NO<sub>2</sub> yellowing only slightly, but not enough to raise Grey Scale ratings above 1-2.

#### 4. Ozonefastness (Table XXIII)

Intratex N had a significant impact on ozonefastness, both alone and as Composition 2. While overall fastness ratings tended to be better at extended cycles compared to the nontreated control, a significant yellowing occurs.

The yellowing of Intratex N overwhelms any improvement achieved by the addition of NH<sub>4</sub>SCN. Samples incorporating NH<sub>4</sub>SCN tend to yellow less when exposed to ozone and higher levels yield more improvement. The significant improvement in ozonefastness of NH<sub>4</sub>SCN alone was not achieved, but were improved over nontreated samples.

#### 5. Benzoyl Peroxide Spotting (Table XXIV)

The dispersant, Tamol SN, had no effect on the benzoyl peroxide spotting performance. Table XXIV shows the benzoyl peroxide performance identical when 0.3% owf NH<sub>4</sub>SCN is applied with either Composition 2 or s.a.c. at several levels.

The performance of NH<sub>4</sub>SCN is not effected at varied s.a.c. levels (as Composition 2 or alone) as shown in Table XXIV.

Benzoyl peroxide spotting improves as the NH<sub>4</sub>SCN concentration is increased from 0.3 to 0.6% owf. The improvement becomes more noticeable at the highest benzoyl peroxide concentration and probably beyond.

### Conclusions

The dispersant, Tamol SN, contributes to the light induced yellowing of Composition 2 but is not the sole cause. Elimination of Tamol SN from Composition 2 would not significantly improve or resolve yellowing on Superba H/S substrates. The elimination of Tamol SN could reduce staining performance slightly at lower add-on's and increase the foaming of the treatment liquor upon spray application.

Intratex N is the sole cause of yellowing upon exposure to NO<sub>2</sub> of Composition 2.

Tamol does not interfere with any of the NH<sub>4</sub>SCN benefits.

Intratex N has a significant impact on ozonefastness (yellows) and overwhelms the ozonefastness improvement benefits of NH<sub>4</sub>SCN. There is, however, a reduction in the yellowing and an improvement over Composition 2 alone at a nominal 0.6% owf NH<sub>4</sub>SCN.

NH<sub>4</sub>SCN has no adverse impacts on Composition 2 stain blocking benefits.

There is a reduction in light induced yellowing when NH<sub>4</sub>SCN is applied with Composition 2. The degree of improvement has varied from marginal to significant during all internal trials. Higher NH<sub>4</sub>SCN levels always yield greater improvement.

Benzoyl peroxide spotting performance may be further improved, particularly at higher benzoyl peroxide concentrations, by increasing the NH<sub>4</sub>SCN level to 0.6% owf.

TABLE XXI

## APPLICATION AND ANALYSIS DATA

| Sample I.D. | Nominal s.a.c. Applied as Comp. 2, % | Nominal s.a.c. Applied* % | Nominal Tamol SN Applied* % | Nominal NH <sub>4</sub> SCN Applied % | pH  | s.a.c. Anal. (As Rec'd) % |
|-------------|--------------------------------------|---------------------------|-----------------------------|---------------------------------------|-----|---------------------------|
| 1           | —                                    | —                         | —                           | —                                     | 7.4 | 0                         |
| 28          | —                                    | —                         | —                           | 0.3                                   | 2.8 | 0                         |
| 2           | 1.0                                  | —                         | —                           | —                                     | 3.5 | 1.05                      |
| 3           | 1.0                                  | —                         | —                           | 0.3                                   | 4.6 | 1.08                      |
| 4           | 1.0                                  | —                         | —                           | 0.6                                   | 4.7 | 1.05                      |
| 5           | 2.0                                  | —                         | —                           | —                                     | 3.1 | 1.91                      |
| 6           | 2.0                                  | —                         | —                           | 0.3                                   | 3.2 | 1.93                      |
| 7           | 2.0                                  | —                         | —                           | 0.6                                   | 3.2 | 2.16                      |
| 8           | 3.0                                  | —                         | —                           | —                                     | 3.0 | 3.19                      |
| 9           | 3.0                                  | —                         | —                           | 0.3                                   | 3.0 | 3.58                      |
| 10          | 3.0                                  | —                         | —                           | 0.6                                   | 3.0 | 3.24                      |
| 11          | 4.0                                  | —                         | —                           | —                                     | 2.8 | 3.23                      |
| 12          | 4.0                                  | —                         | —                           | 0.3                                   | 2.9 | 4.20                      |
| 13          | 4.0                                  | —                         | —                           | 0.6                                   | 2.9 | 3.90                      |
| 14          | —                                    | 2.0                       | —                           | —                                     | 3.2 | 2.10                      |
| 15          | —                                    | 2.0                       | —                           | 0.3                                   | 3.2 | 2.43                      |
| 16          | —                                    | 3.0                       | —                           | —                                     | 2.9 | 3.83                      |
| 17          | —                                    | 3.0                       | —                           | 0.3                                   | 2.8 | 4.20                      |
| 18          | —                                    | 4.0                       | —                           | —                                     | 2.7 | 4.97                      |
| 19          | —                                    | 4.0                       | —                           | 0.3                                   | 2.7 | 4.73                      |
| 20          | —                                    | —                         | 1.93                        | —                                     | 2.9 | —                         |
| 21          | —                                    | —                         | 1.93                        | 0.3                                   | 2.9 | —                         |
| 22          | —                                    | —                         | 2.90                        | —                                     | 2.8 | —                         |
| 23          | —                                    | —                         | 2.90                        | 0.3                                   | 2.8 | —                         |
| 24          | —                                    | —                         | 3.89                        | —                                     | 2.8 | —                         |
| 25          | —                                    | —                         | 3.89                        | 0.3                                   | 2.9 | —                         |

\*Materials applied as supplied, not blended or part of a composition.

## Notes:

Carpet temperature before A/T ranged from 132 to 144° F. (55.6–62.2° C.).

A/T liquor temperature was 178 to 183° F. (55.6–62.2° C.).

Actual temperature after A/T ranged from 158 to 172° F. (70–77.8° C.).

TABLE XXII

| Sample I.D. | STAINING PERFORMANCE DATA                                                     |      |      |      |      |      |
|-------------|-------------------------------------------------------------------------------|------|------|------|------|------|
|             | Stain Rating (0 = best, 10 = worst)<br>Time Before Blotting With Water, Hours |      |      |      |      |      |
|             | 0.05                                                                          | 0.5  | 1    | 4    | 8    | 24   |
| 1           | 9.5                                                                           | 9.5  | 9.5  | 9.5  | 9.5  | 9.5  |
| 2           | 0                                                                             | 1.0  | 2.0  | 3.5  | 3.5  | 3.5  |
| 3           | 0                                                                             | 1.0  | 1.5  | 2.0  | 3.0  | 3.0  |
| 4           | 0                                                                             | 0.5  | 0.75 | 1.5  | 1.0  | 1.0  |
| 5           | 0                                                                             | 0.25 | 0.5  | 1.0  | 1.0  | 1.5  |
| 6           | 0                                                                             | 0.25 | 0.25 | 1.0  | 1.0  | 1.0  |
| 7           | 0                                                                             | 0    | 0.25 | 0.5  | 0.5  | 0.5  |
| 8           | 0                                                                             | 0.25 | 0.25 | 0.75 | 0.75 | 0.75 |
| 9           | 0                                                                             | 0    | 0.10 | 0.25 | 0.25 | 0.25 |
| 10          | 0                                                                             | 0    | 0    | 0.25 | 0.5  | 0.5  |
| 11          | 0                                                                             | 0    | 0.1  | 0.5  | 0.25 | 0.5  |
| 12          | 0                                                                             | 0    | 0.1  | 0.25 | 0.25 | 0.5  |
| 13          | 0                                                                             | 0    | 0    | 0.25 | 0.25 | 0.25 |
| 14          | 0                                                                             | 0.5  | 1.0  | 1.5  | 2.0  | 3.0  |
| 15          | 0                                                                             | 0.5  | 1.0  | 1.25 | 2.0  | 2.5  |
| 16          | 0                                                                             | 0.25 | 0.25 | 0.5  | 0.5  | 0.5  |
| 17          | 0                                                                             | 0    | 0.25 | 0.5  | 0.25 | 0.25 |
| 18          | 0                                                                             | 0.1  | 0.1  | 0.25 | 0.25 | 0.25 |
| 19          | 0                                                                             | 0    | 0    | 0.25 | 0.1  | 0.1  |

35

TABLE XXIII-continued

| Sample I.D. | COLORFASTNESS DATA |                   |                   |     |     |     |
|-------------|--------------------|-------------------|-------------------|-----|-----|-----|
|             | Grey Scale Rating  |                   |                   |     |     |     |
|             | Lightfastness, AFU | Ozonefastness, cy | NO <sub>2</sub> * |     |     |     |
|             | 20                 | 40                | 1                 | 2   | 3   | 5   |
| 9           | 2.0                | 2.5               | 2.5               | 2.5 | 2.5 | 2.0 |
| 10          | 2.5                | 2.5               | 3.0               | 3.0 | 2.5 | 2.5 |
| 11          | 2.0                | 2.0               | 2.5               | 2.5 | 2.0 | 2.0 |
| 12          | 2.0                | 2.0               | 2.5               | 2.5 | 2.0 | 2.0 |
| 13          | 2.5                | 2.5               | 3.0               | 3.0 | 2.5 | 2.5 |
| 14          | 2.5                | 2.5               | 2.5               | 2.5 | 2.0 | 2.0 |
| 15          | 3.0                | 2.5               | 2.5               | 2.5 | 2.0 | 2.0 |
| 16          | 2.0                | 2.0               | 2.5               | 2.5 | 2.0 | 2.0 |
| 17          | 2.5                | 2.5               | 2.5               | 2.5 | 2.5 | 2.0 |
| 18          | 2.0                | 2.0               | 2.0               | 2.0 | 2.0 | 2.0 |
| 19          | 2.5                | 2.0               | 2.5               | 2.5 | 2.0 | 2.0 |
| 20          | 2.5                | 2.5               | 2.5               | 2.5 | —   | —   |
| 21          | 2.5                | 2.5               | 3.0               | 3.0 | —   | —   |
| 22          | 2.0                | 2.0               | 3.0               | 2.5 | —   | —   |
| 23          | 2.0                | 2.0               | 3.0               | 2.5 | —   | —   |
| 24          | 2.0                | 2.0               | 3.0               | 2.5 | —   | —   |
| 25          | 2.0                | 2.0               | 3.0               | 2.5 | —   | —   |

\*High R.H. nitrogen dioxide (AATCC TM-164).

55

TABLE XXIII

| Sample I.D. | COLORFASTNESS DATA |                   |                   |     |     |     |
|-------------|--------------------|-------------------|-------------------|-----|-----|-----|
|             | Grey Scale Rating  |                   |                   |     |     |     |
|             | Lightfastness, AFU | Ozonefastness, cy | NO <sub>2</sub> * |     |     |     |
|             | 20                 | 40                | 1                 | 2   | 3   | 5   |
| 1           | 4.0                | 3.0               | 3.0               | 2.5 | 2.0 | 1.0 |
| 28          | 4.0                | 3.0               | 3.5               | 3.0 | 3.0 | 3.0 |
| 2           | 2.5                | 3.0               | 3.0               | 2.5 | 2.0 | 1.5 |
| 3           | 3.0                | 3.5               | 3.0               | 2.5 | 2.5 | 1.5 |
| 4           | 3.5                | 3.5               | 3.0               | 2.5 | 2.5 | 1.5 |
| 5           | 2.5                | 2.5               | 2.5               | 2.0 | 2.0 | 1.5 |
| 6           | 2.5                | 2.5               | 2.5               | 2.5 | 2.0 | 1.5 |
| 7           | 3.0                | 3.0               | 3.0               | 2.5 | 2.5 | 1.5 |
| 8           | 2.0                | 2.5               | 2.5               | 2.0 | 2.0 | 1.5 |

60

TABLE XXIV

| Sample I.D. | BENZOYL PEROXIDE SPOTTING DATA*                                                            |      |      |      |     |
|-------------|--------------------------------------------------------------------------------------------|------|------|------|-----|
|             | Spot Visibility (0 = Invisible; 10 = Bright)<br>Benzoyl Peroxide Conc., % Soln. in Acetone |      |      |      |     |
|             | 0.005                                                                                      | 0.01 | 0.05 | 0.1  | 1.0 |
| 1           | 0.5                                                                                        | 1.5  | 6.5  | 8.0  | 9.0 |
| 28          | 0                                                                                          | 0    | 0.75 | 1.0  | 8.0 |
| 2           | 0.25                                                                                       | 2.0  | 6.75 | 8.0  | 8.5 |
| 3           | 0                                                                                          | 0    | 1.25 | 4.0  | 7.0 |
| 4           | 0                                                                                          | 0    | 0.25 | 0.5  | 2.0 |
| 5           | 0.5                                                                                        | 1.75 | 5.5  | 6.5  | 7.5 |
| 6           | 0                                                                                          | 0    | 0.5  | 1.0  | 2.0 |
| 7           | 0                                                                                          | 0    | 0.1  | 0.75 | 3.0 |
| 8           | 0.25                                                                                       | 2.0  | 7.25 | 7.5  | 7.5 |
| 9           | 0                                                                                          | 0    | 0.5  | 1.25 | 2.0 |

TABLE XXIV-continued

| Sample | BENZOYL PEROXIDE SPOTTING DATA*              |      |      |      |      |
|--------|----------------------------------------------|------|------|------|------|
|        | Spot Visibility (0 = Invisible; 10 = Bright) |      |      |      |      |
|        | Benzoyl Peroxide Conc., % Soln. in Acetone   |      |      |      |      |
| I.D.   | 0.005                                        | 0.01 | 0.05 | 0.1  | 1.0  |
| 10     | 0                                            | 0    | 0.25 | 0.5  | 0.75 |
| 11     | 1.0                                          | 2.5  | 7.5  | 8.0  | 8.5  |
| 12     | 0                                            | 0    | 0.5  | 1.0  | 3.0  |
| 13     | 0                                            | 0    | 0.1  | 0.5  | 1.25 |
| 14     | 0.5                                          | 1.5  | 6.5  | 7.5  | 8.0  |
| 15     | 0                                            | 0    | 0.5  | 1.0  | 2.0  |
| 16     | —                                            | —    | —    | —    | —    |
| 17     | —                                            | —    | —    | —    | —    |
| 18     | 0.25                                         | 1.0  | 6.5  | 7.5  | 8.5  |
| 19     | 0                                            | 0    | 0.5  | 0.75 | 1.75 |

\*Sample spotted with 1 ml of benzoyl peroxide solution and exposed in chamber at 90° F. (32.2° C.) and 80% R.H. for three days.

### EXAMPLE 6

This example demonstrates the two-step, batch-batch (beck-beck) process embodiment of this invention.

Prior art has shown that application of sulfonated aromatic condensates (stain blockers) to nylon improves resistance to staining by most food colors. In the prior art, the preferred mode of application has been a low temperature (120° to 180° F. (48.9° to 82.2° C.) treatment with the stain blocker after dyeing has been completed. Also, prior art includes application of stain blockers concurrent with dye application. This invention embodies application of a portion of the total stain blocker concurrently with dye application, and application of the remainder in a low temperature aftertreatment step. (two-step process).

The two-step process results in a level of stain performance superior to that which is achieved by the prior art at the same total add-on concentration of stain blocker. In addition, use of ammonium thiocyanate in the aftertreatment step improves dye fastness to ozone, benzoyl peroxide (acne medications) and light.

It is theorized that the improvement over prior art is achieved by maximization of the concentration of stain blocker in a thin zone near the fiber surface and that this condition results in better stain resistance. The two-step process promotes this condition by sorption of a portion of the stain blocker during the dyeing operation which is fully penetrated into the cross-section of the nylon fiber. The sorption of the portion of stain blocker subsequently applied in the low temperature aftertreatment step is retarded by the presence of the existing portion already on the fiber, therefore, increasing the effective concentration near the fiber surface. The presence of magnesium sulfate in both steps of the process accelerates rate of sorption of the stain blocker by increasing the bath electrolyte concentration and by complexing with the stain blockers thus reducing molecular mobility in the nylon.

#### Example 6—Part 1

This example shows that two-step process is superior to either concurrent or aftertreatment.

##### Carpet Fabric

###### 1185 denier fluorocarbon treated Superba Heat Set

##### Process

A total of 2.0% owf Intratex N was applied to carpet. The total was distributed between dyebath and aftertreatment in the following ways:

| 5 | Dyebath, % | Aftertreatment, % |     |
|---|------------|-------------------|-----|
|   |            | 0                 | 100 |
|   |            | 50                | 50  |
|   |            | 100               | 0   |

Varying amounts of Magnesium Sulfate were used (0% owf to 4% owf).

10 Dyebath conditions were typical of industry practice.

Dyeing procedure as follows:

1. Load fabric and wet out at 20:1 Liquor Ratio

2. Add 1.0% owf Dowfax 2Al-sodium mono-and didodecyl disulfonated diphenyl oxide (45% active)

3. Add the specified amount of Intratex N-1

4. Add the specified amount of Magnesium Sulfate

5. Run 5 minutes

6. Add 0.5% Sequestrene 30A (EDTA) or equiv.

7. Add 1% owf ammonium sulfate

8. Add 0.5% owf ammonium hydroxide

9. Add predissolved dyes

10. Run 10 minutes

11. Raise temperature to boil

12. Boil 30 minutes

13. Drop and rinse cold

14. Aftertreat if indicated

Aftertreatment procedure as follows:

1. Refill Beck at 20:1 Liquor Ratio

2. Add specified amount of Magnesium Sulfate

3. Add specified amount of Intratex N1

4. Run 10 minutes

5. Lower pH to 2.0 to 2.1 with sulfamic acid

6. Raise temperature to 160° F. (71.1° C.).

7. Hold at temperature 20 minutes

8. Drop bath and rinse cold

##### Performance

Reference samples Nos. 17 through 31 in Table XXV. Samples 23, 24 and 25 prepared with the 50%/50% two-step process are superior. Those samples which passed the dip test were further tested by the drop test.

##### Test Protocols:

1. "Dip Test"—Immerse a 5 gram sample of unfinished carpet into a large excess of Cherry Kool-Aid (unsweetened) at room temperature for 30 minutes. Rinse with cold water, dry and assess tie stain.

2. "Drop Test"—Drop 30 ml. Cherry Kool-Aid<sup>1</sup> (unsweetened) onto the finished carpet from a height of

50 12 inches. Allow to stand for seven hours. Blot with paper towels using water spray to aid in removal.

<sup>1</sup> Registered TM of General Foods Corporation.

#### Example 6—Part 2

This example shows use of ammonium thiocyanate in two-step process for improved resistance to benzoyl peroxide and light fading.

##### Carpet Fabric

###### 60 1700 denier Superba Heat Set (High ICP fiber)

##### Process

Using the process of Part 1, a total of 2.8% Intratex N was applied using the 50%/50% two-step mode. A 65 second sample was prepared in the same way but an Intratex N pre-formulated mixture containing ammonium thiocyanate (Composition 3) was used in the aftertreatment step. Composition 3 is 40% Intratex N-1, 12%

ammonium thiocyanate, 21.5% Monawet MB45, 26.5% Water.

Performance

Reference samples "H" and "I" in Tables XXVI to 5 XXVIII. Using the "Drop Test" Protocol from Example 1, sample "I" has good stain resistance (somewhat poorer than "H") but very significant improvements in benzoyl peroxide and light fading.

Example 6—Part 3

This example shows that 50%/50% two-step mode is preferred and the 2% magnesium sulfate is optimum.

Carpet Fabric

1185 denier fluorocarbon treated autoclave Heat Set (high ICP fiber)

Process

Using the process of Part 1, a total of 3.0% Intratex N-1 was applied using the two-step mode.

The total was distributed between dyebath and after-treatment in the following ways:

TABLE XXV-continued

|    |     |     |     |     |   |
|----|-----|-----|-----|-----|---|
| 25 | 1.0 | 2.0 | 1.0 | 4.0 | P |
| 26 | 1.0 | 4.0 | 1.0 | 0   | S |
| 27 | 1.0 | 4.0 | 1.0 | 2.0 | P |
| 28 | 1.0 | 4.0 | 1.0 | 4.0 | P |
| 29 | 2.0 | 0   | —   | —   | F |
| 30 | 2.0 | 2.0 | —   | —   | F |
| 31 | 2.0 | 4.0 | —   | —   | F |
| 32 | 0   | 0   | 2.8 | 0   | F |
| 33 | 0   | 0   | 2.8 | 2.0 | F |
| 34 | 0   | 0   | 2.8 | 4.0 | F |
| 35 | 1.4 | 0   | 1.4 | 0   | F |
| 36 | 1.4 | 0   | 1.4 | 2.0 | F |
| 37 | 1.4 | 0   | 1.4 | 4.0 | F |
| 38 | 1.4 | 2.0 | 1.4 | 0   | S |
| 39 | 1.4 | 2.0 | 1.4 | 2.0 | P |
| 40 | 1.4 | 2.0 | 1.4 | 4.0 | P |
| 41 | 1.4 | 4.0 | 1.4 | 0   | P |
| 42 | 1.4 | 4.0 | 1.4 | 2.0 | P |
| 43 | 1.4 | 4.0 | 1.4 | 4.0 | P |
| 44 | 2.8 | 0   | —   | —   | F |
| 45 | 2.8 | 2.0 | —   | —   | P |
| 46 | 2.8 | 4.0 | —   | —   | P |

\*Epsom salt

\*\*Kool Aid

\*\*\*P = Pass (No Stain)

F = Fail (Noticeably Stained)

S = Slight Stain (Just Detectable)

| Dyebath, % | Aftertreatment, % | Gray Scale |                           |                             |
|------------|-------------------|------------|---------------------------|-----------------------------|
|            |                   | No.        | 7-Hour Kool-Aid Staining* | Xenon Light-Fastness 20 AFU |
| 0          | 100               | 1          | 7.5                       | 3.0                         |
| 5          | 95                | 2          | —                         | 3.0                         |
| 10         | 90                | 3          | —                         | 3.0                         |
| 20         | 80                | 4          | —                         | 3.5                         |
| 30         | 70                | 5          | —                         | 3.0                         |
| 50         | 50                | 6          | —                         | 2.5                         |
|            |                   | 7          | —                         | 3.0                         |
|            |                   | 8          | 1.5                       | 3.5                         |
|            |                   | 9          | 0.75                      | 3.5                         |
|            |                   | 10         | 1.0                       | 3.5                         |
|            |                   | 11         | 1.0                       | 3.5                         |
|            |                   | 12         | 0.75                      | 3.5                         |
|            |                   | 13         | 0.25                      | 4.0                         |
|            |                   | 14         | —                         | 2.5                         |
|            |                   | 15         | —                         | 2.0                         |
|            |                   | 16         | 1.0                       | 3.0                         |
|            |                   | 17         | —                         | 4.0                         |
|            |                   | 18         | —                         | 3.5                         |
|            |                   | 19         | —                         | 4.0                         |
|            |                   | 20         | —                         | 4.0                         |
|            |                   | 21         | —                         | 3.5                         |
|            |                   | 22         | —                         | 3.5                         |
|            |                   | 23         | 0.5                       | 4.0                         |
|            |                   | 24         | 0                         | 3.5                         |
|            |                   | 25         | 0.1                       | 3.5                         |
|            |                   | 26         | 0.5                       | 3.5                         |
|            |                   | 27         | 0                         | 3.0                         |
|            |                   | 28         | 0                         | 3.0                         |
|            |                   | 29         | —                         | 2.5                         |
|            |                   | 30         | —                         | 2.5                         |
|            |                   | 31         | —                         | 2.5                         |
|            |                   | 32         | —                         | 3.5                         |
|            |                   | 33         | —                         | 4.0                         |
|            |                   | 34         | —                         | 4.0                         |
|            |                   | 35         | —                         | 2.5                         |
|            |                   | 36         | —                         | 2.5                         |
|            |                   | 37         | —                         | 2.5                         |
|            |                   | 38         | 0.5                       | 2.0                         |
|            |                   | 39         | 0.1                       | 2.5                         |
|            |                   | 40         | 0                         | 2.5                         |
|            |                   | 41         | 0                         | 3.0                         |
|            |                   | 42         | 0                         | 3.0                         |
|            |                   | 43         | 0                         | 3.0                         |
|            |                   | 44         | —                         | 2.0                         |
|            |                   | 45         | 0.1                       | 2.5                         |
|            |                   | 46         | 0.1                       | 3.0                         |

Varying amounts of magnesium sulfate were used 35 (0% owf to 4% owf)

Performance

Reference samples 2 through 23 Table XXIX. Using the test protocols from Example 1, samples 20 through 40 (50%/50% application mode) have best stain resistance. Sample 20 is best of group (uses 2% and 2% owf magnesium sulfate).

TABLE XXV

| No. | Dyebath |     | Aftertreatment |     | K/A** "Dip" Test*** | 45 |
|-----|---------|-----|----------------|-----|---------------------|----|
|     | s.a.c.  | ES* | s.a.c.         | ES* |                     |    |
| 1   | 0       | 0   | —              | —   | F                   |    |
| 2   | 0       | 0   | 1.6            | 0   | F                   |    |
| 3   | 0       | 0   | 1.6            | 2.0 | F                   |    |
| 4   | 0       | 0   | 1.6            | 4.0 | F                   |    |
| 5   | 0.8     | 0   | 0.8            | 0   | F                   |    |
| 6   | 0.8     | 0   | 0.8            | 2.0 | F                   |    |
| 7   | 0.8     | 0   | 0.8            | 4.0 | F                   |    |
| 8   | 0.8     | 2.0 | 0.8            | 0   | S                   |    |
| 9   | 0.8     | 2.0 | 0.8            | 2.0 | P                   |    |
| 10  | 0.8     | 2.0 | 0.8            | 4.0 | S                   |    |
| 11  | 0.8     | 4.0 | 0.8            | 0   | S                   |    |
| 12  | 0.8     | 4.0 | 0.8            | 2.0 | S                   |    |
| 13  | 0.8     | 4.0 | 0.8            | 4.0 | P                   |    |
| 14  | 1.6     | 0   | —              | —   | F                   |    |
| 15  | 1.6     | 2.0 | —              | —   | F                   |    |
| 16  | 1.6     | 4.0 | —              | —   | S                   |    |
| 17  | 0       | 0   | 2.0            | 0   | F                   |    |
| 18  | 0       | 0   | 2.0            | 2.0 | F                   |    |
| 19  | 0       | 0   | 2.0            | 4.0 | F                   |    |
| 20  | 1.0     | 0   | 1.0            | 0   | F                   |    |
| 21  | 1.0     | 0   | 1.0            | 2.0 | F                   |    |
| 22  | 1.0     | 0   | 1.0            | 4.0 | F                   |    |
| 23  | 1.0     | 2.0 | 1.0            | 0   | P                   |    |
| 24  | 1.0     | 2.0 | 1.0            | 2.0 | P                   |    |

\*Drop test

TABLE XXVI

| No. | Description                 | Original Samples Before Blot, Hours** |      |      |      | s.a.c. by analysis % | Steam Cleaned Before Blot, Hours |      |      |      |
|-----|-----------------------------|---------------------------------------|------|------|------|----------------------|----------------------------------|------|------|------|
|     |                             | 1                                     | 4    | 7    | 24   |                      | 1                                | 4    | 7    | 24   |
| A   | Control                     | 7.50                                  | 8.00 | 8.00 | 8.00 | —                    | —                                | —    | —    | —    |
|     | <u>Aftertreatments</u>      |                                       |      |      |      |                      |                                  |      |      |      |
| B   | 5.0% Intratex N-1 + 4% ES*  | 0.10                                  | 0.25 | 0.50 | 0.50 | 13.58***             | 2.00                             | 3.50 | 3.00 | 3.50 |
| C   | 10% Composition 3           | 0.75                                  | 1.00 | 1.50 | 1.00 | 4.45                 | 2.50                             | 4.00 | 3.50 | 4.00 |
| D   | 10% Composition 3 + 4% ES   | 0.75                                  | 1.00 | 1.00 | 1.50 | 4.64                 | 4.00                             | 3.00 | 4.00 | 4.00 |
| E   | 12.5% Composition 3         | 0.25                                  | 1.00 | 1.00 | 1.50 | 5.83                 | 1.50                             | 4.50 | 3.50 | 4.00 |
|     | <u>Two-Step</u>             |                                       |      |      |      |                      |                                  |      |      |      |
| F   | 1.0% Intratex N-1 + 2.0% ES | 1.0% Intratex + 2.0% ES               | 4.50 | 3.50 | 4.00 | 3.00                 | 1.69                             | 6.00 | 5.50 | 6.50 |
| G   | 1.4% Intratex N-1 + 2.0% ES | 1.4% Intratex + 4.0% ES               | 1.00 | 2.00 | 2.00 | 1.50                 | 2.14                             | 4.00 | 4.00 | 5.00 |
| H   | 1.4% Intratex N-1 + 4.0% ES | 1.4% Intratex + 4.0% ES               | 0.10 | 0.10 | 0.25 | 0.50                 | 2.57                             | 5.50 | 4.50 | 4.50 |
| I   | 1.4% Intratex N-1 + 2.0% ES | 3.5% Comp. 3 + 4.0% ES                | 1.00 | 1.00 | 1.50 | 0.75                 | 2.14                             | 4.00 | 5.00 | 4.50 |

\*ES—Epsom salt

\*\*Drop test 0 = best 10 worst

\*\*\*Error in application

Note: All aftertreatments at pH = 2, 160° F. (°C.).

TABLE XXVII

| No. | Spot Visibility* Benzoyl Peroxide Spotting Data |      |      |      |      |
|-----|-------------------------------------------------|------|------|------|------|
|     | 0.005                                           | 0.01 | 0.05 | 0.1  | 1.0  |
| A   | 3.50                                            | 6.50 | 7.50 | 9.00 | 9.00 |
| B   | 3.00                                            | 6.50 | 7.50 | 8.00 | 8.00 |
| C   | 0                                               | 0.50 | 1.00 | 2.00 | 2.50 |
| D   | 0                                               | 0.25 | 1.00 | 3.00 | 3.00 |
| E   | 0                                               | 0.10 | 0.75 | 1.50 | 1.00 |
| F   | 3.00                                            | 6.50 | 7.50 | 8.00 | 9.00 |
| G   | 4.50                                            | 6.50 | 7.50 | 8.00 | 8.50 |
| H   | 4.00                                            | 6.00 | 7.00 | 8.00 | 8.50 |
| I   | 0.25                                            | 0.75 | 1.50 | 3.00 | 3.00 |

\*0 = Invisible; 10 = Bright

TABLE XXVIII

| No. | Gray Scale Rating  |     |     |       |     |     |
|-----|--------------------|-----|-----|-------|-----|-----|
|     | Lightfastness, AFU |     |     | No. 2 |     |     |
|     | 20                 | 40  | 60  | 1     | 2   | 1   |
| A   | 4                  | 3   | 2-3 | 3-4   | 2-3 | 2   |
| B   | 3                  | 2-3 | 2-3 | 4-5   | 4   | 2   |
| C   | 4                  | 3-4 | 3   | 4-5   | 4   | 2-3 |
| D   | 4                  | 3-4 | 3   | 4     | 3-4 | 3-4 |
| E   | 4                  | 3-4 | 3   | 4-5   | 4   | 3   |
| F   | 4-5                | 4   | 4   | 4-5   | 4   | 2-3 |
| G   | 4                  | 3-4 | 3   | 4     | 3-4 | 2-3 |
| H   | 3-4                | 3   | 3   | 4     | 3-4 | 2   |
| I   | 4                  | 3   | 3-4 | 4     | 3-4 | 3   |

TABLE XXIX

| No. | Dyebath % ofw |     | Aftertreat % ofw |     | K/A Dip Test** |
|-----|---------------|-----|------------------|-----|----------------|
|     | s.a.c.        | ES* | s.a.c.           | ES* |                |
| 1   | 0             | 0   | —                | —   | 23             |
| 2   | 0             | 0   | 3.0              | 2.0 | 22             |
| 3   | 0             | 0   | 3.0              | 4.0 | 21             |
| 4   | 0.15          | 2.0 | 2.85             | 2.0 | 20             |
| 5   | 0.15          | 2.0 | 2.85             | 4.0 | 17             |
| 6   | 0.15          | 4.0 | 2.85             | 2.0 | 13             |
| 7   | 0.15          | 4.0 | 2.85             | 4.0 | 16             |
| 8   | 0.3           | 2.0 | 2.7              | 2.0 | 14             |
| 9   | 0.3           | 2.0 | 2.7              | 4.0 | 18             |
| 10  | 0.3           | 4.0 | 2.7              | 2.0 | 12             |
| 11  | 0.3           | 4.0 | 2.7              | 4.0 | 15             |
| 12  | 0.6           | 2.0 | 2.4              | 2.0 | 9              |
| 13  | 0.6           | 2.0 | 2.4              | 4.0 | 19             |
| 14  | 0.6           | 4.0 | 2.4              | 2.0 | 10             |
| 15  | 0.6           | 4.0 | 2.4              | 4.0 | 11             |
| 16  | 0.9           | 2.0 | 2.1              | 2.0 | 7              |
| 17  | 0.9           | 2.0 | 2.1              | 4.0 | 8              |
| 18  | 0.9           | 4.0 | 2.1              | 2.0 | 5              |
| 19  | 0.9           | 4.0 | 2.1              | 4.0 | 6              |

TABLE XXIX-continued

| No. | 7-Hour Kool-Aid Staining* |      | Xenon Lightfastness 20 AFU |     | s.a.c. by analysis % |      |
|-----|---------------------------|------|----------------------------|-----|----------------------|------|
|     | 20                        | 1.5  | 2.0                        | 1.5 | 2.0                  | 1    |
| 25  | 20                        | 1.5  | 2.0                        | 1.5 | 4.0                  | 4    |
|     | 21                        | 1.5  | 2.0                        | 1.5 | 4.0                  | 4    |
|     | 22                        | 1.5  | 4.0                        | 1.5 | 2.0                  | 2    |
|     | 23                        | 1.5  | 4.0                        | 1.5 | 4.0                  | 3    |
| 30  | 1                         | 7.50 | 3-4                        | —   | —                    | —    |
|     | 2                         | 2.50 | 4                          | 4   | 3.78                 | 3.78 |
|     | 3                         | 3.00 | 4                          | 4-5 | 3.93                 | 3.93 |
|     | 4                         | 1.00 | 4                          | 5   | 3.38                 | 3.38 |
|     | 5                         | 1.50 | 3-4                        | 5   | 3.48                 | 3.48 |
| 35  | 6                         | 1.50 | 4                          | 4-5 | 3.38                 | 3.38 |
|     | 7                         | 1.50 | 4                          | 4-5 | 3.60                 | 3.60 |
|     | 8                         | 1.00 | 4-5                        | 4-5 | 3.60                 | 3.60 |
|     | 9                         | 1.50 | 3                          | 4   | 3.60                 | 3.60 |
|     | 10                        | 1.00 | 3-4                        | 4   | 3.38                 | 3.38 |
|     | 11                        | 1.50 | 3                          | 4-5 | 3.29                 | 3.29 |
|     | 12                        | 1.00 | 4                          | 4-5 | 3.24                 | 3.24 |
|     | 13                        | 1.00 | 3-4                        | 4   | 3.00                 | 3.00 |
|     | 14                        | 1.50 | 4                          | 4-5 | 3.15                 | 3.15 |
|     | 15                        | 1.50 | 3-4                        | 4   | 3.22                 | 3.22 |
|     | 16                        | 0.75 | 3                          | 4   | 3.15                 | 3.15 |
|     | 17                        | 0.50 | 3-4                        | 4-5 | 3.00                 | 3.00 |
|     | 18                        | 0.75 | 4                          | 4-5 | 3.03                 | 3.03 |
|     | 19                        | 1.00 | 3-4                        | 4   | 3.10                 | 3.10 |
|     | 20                        | 0.10 | 3-4                        | 4   | 2.72                 | 2.72 |
|     | 21                        | 0.50 | 3-4                        | 4   | 2.86                 | 2.86 |
|     | 22                        | 0.10 | 3-4                        | 4   | 2.82                 | 2.82 |
|     | 23                        | 0.75 | 3                          | 4-5 | 2.91                 | 2.91 |

\*drop test

## EXAMPLE 7

This example describes use of a sequestering agent in the continuous aftertreatment process of this invention. The general procedure was as in Example 2.

## Experimental Summary

## Substrate

60 1185 denier fluorocarbon treated Superba H/S in 32 ounce per square yard cut pile fabric construction and beck dyed into Argent Grey shade.

Continuously aftertreated using nominal add-on 15.9% ofw Compositon 2 (3.0% ofw Intratex N) with no additional pH adjustment (actual pH 2.9).

65 Calquest ADP (Mfrs. Chem.) added to treatment bath containing Comp. 2 at levels corresponding to 0.5 and 1.0% ofw.

## Standard Continuous Process

Prewet/heat carpet at 195° F. (90.6° C.) and 100% w.p.u. to achieve a carpet temperature prior to treatment of 135° to 140° F. (57.2° to 60° C.).

## Conclusions

The use of sequestering agent in the Composition 2 formulation shows reduced yellowing a low lightfastness exposures and upon exposure to ozone.

TABLE XXX

| Sam-<br>ple | EFFECT OF SEQUESTERING AGENTS ON LIGHT INDUCED<br>YELLOWING (NOMINAL 3.0% OFW INTRATEX N<br>ANALYSIS, STAINING PERFORMANCE,<br>CHANGE-OF-SHADE AND COLORFASTNESS DATA) |                                    |                                |                                           |     |      |     |     |     |        | Grey Scale Rating |                            |     |                           |     |                                        |  |
|-------------|------------------------------------------------------------------------------------------------------------------------------------------------------------------------|------------------------------------|--------------------------------|-------------------------------------------|-----|------|-----|-----|-----|--------|-------------------|----------------------------|-----|---------------------------|-----|----------------------------------------|--|
|             | Nominal<br>Comp. 2<br>Conc.,                                                                                                                                           | Nominal<br>Seq.<br>Agent<br>Conc., | Intratex<br>N Ana-<br>lyzed, % | Stain Rating<br>(0 = best, 10 = worst)    |     |      |     |     |     |        | Shade<br>Change   | Light-<br>fastness,<br>AFU |     | Ozone-<br>fastness,<br>cy |     | NO <sub>2</sub> ***<br>Fastness,<br>cy |  |
|             |                                                                                                                                                                        |                                    |                                | Time Before Blotting<br>With Water, Hours |     |      |     |     |     |        |                   | 20                         |     | 60                        |     | 1                                      |  |
|             |                                                                                                                                                                        |                                    |                                | 0.05                                      | 0.5 | 1    | 4   | 8   | 24  | 20     |                   | 60                         | 1   | 2                         | 1   |                                        |  |
| 1           | N.T.                                                                                                                                                                   | —                                  | 0                              | 7.0                                       | 8.5 | 8.50 | 8.5 | 8.5 | 8.5 | —      | 3.5               | 2.5                        | 3.0 | 2.5                       | 2.5 |                                        |  |
| 2           | 3.0                                                                                                                                                                    | —                                  | 4.22                           | 0                                         | 0   | 0    | 0.1 | 0.1 | 0.1 | M(B)   | 2.5               | 3.0                        | 3.0 | 2.5                       | 1.0 |                                        |  |
| 3           | 3.0                                                                                                                                                                    | 0.5                                | 3.41                           | 0                                         | 0   | 0    | 0.1 | 0.1 | 0.1 | M-Y(B) | 3.5               | 4.0                        | 3.0 | 3.0                       | 1.5 |                                        |  |
| 4           | 3.0                                                                                                                                                                    | 1.0                                | 3.66                           | 0                                         | 0   | 0    | 0.1 | 0.1 | 0.1 | M-Y(B) | 3.5               | 3.5                        | 3.0 | 3.0                       | 1.5 |                                        |  |

\*Calquest ADP (Manufacturers Chemical)

\*\*N.T. = Not treated

\*\*\*High R.H. Nitrogen Dioxide. AATCC TM-164.

Apply A/T liquor at 400% w.p.u. and 175° to 180° F. (79.4° to 82.2° C.) to achieve a post-A/T carpet temperature of 160° to 170° F. (71.1° to 76.7° C.).

After treatment, 30-second dwell time before washing (at 40:1 liquor ratio), hydroextraction and drying.

25

Other sequestering agents would also be useful, for example, the polyphosphates, such as Calgon which is sodium hexametaphosphate, aminocarboxylic acids, such as EDTA or ethylenediaminetetraacetic acid, the amino alcohols, and the hydroxycarboxylic acids, including citric acid.

TABLE XXXI

ADDITION OF SEQUESTERING AGENTS TO  
INHIBIT LIGHT INDUCED YELLOWING  
(1185 Fluorocarbon Treated Superba Substrate,  
Nominal 15.9% ofw Composition 2-3.0% Intratex N)  
Analysis and Colorfastness Data

| Sample | I.D.                       | Additives | A/T pH | s.a.c. | Grey Scale Rating     |     |     |                      |     |     |                                     |
|--------|----------------------------|-----------|--------|--------|-----------------------|-----|-----|----------------------|-----|-----|-------------------------------------|
|        |                            |           |        |        | Lightfastness,<br>AFU | 20  | 40  | Ozonefastness,<br>cy | 1   | 2   | NO <sub>2</sub> * Fast-<br>ness, cy |
| 1      | Not Treated                | —         | —      | 0      | 5.0                   | 4.5 | 3.0 | 2.5                  | 2.5 | 2.5 | 2.5                                 |
| 2      | No Additive (Comp. 2 only) | 3.0       | 2.46   | 3.0    | 3.5                   | 3.5 | 3.5 | 3.0                  | 3.0 | 1.5 | 1.5                                 |
| 3      | 0.50% ofw Calquest ADP     | 3.3       | 2.95   | 3.0    | 3.5                   | 4.0 | 3.5 | 3.0                  | 3.0 | 2.0 | 2.0                                 |
| 4      | 0.10% ofw Sequestrene 30A  | 3.2       | 2.75   | 4.0    | 4.0                   | 4.0 | 3.5 | 3.0                  | 3.0 | 2.0 | 2.0                                 |
| 5      | 0.25% ofw Sequestrene 30A  | 3.7       | 3.02   | 4.0    | 3.5                   | 4.0 | 3.5 | 3.0                  | 3.0 | 2.0 | 2.0                                 |
| 6      | 0.50% ofw Sequestrene 30A  | 3.3**     | 2.54   | 4.0    | 3.5                   | 3.5 | 3.5 | 3.0                  | 3.0 | 2.0 | 2.0                                 |
| 7      | 0.10% ofw SHMP*            | 3.0       | 2.80   | 4.0    | 3.5                   | 3.5 | 3.5 | 3.0                  | 3.0 | 2.0 | 2.0                                 |
| 8      | 0.25% ofw SHMP*            | 3.3       | 2.95   | 3.5    | 3.5                   | 3.5 | 3.0 | 2.5                  | 2.5 | 2.0 | 2.0                                 |
| 9      | 0.50% ofw SHMP*            | 3.6       | 3.09   | 3.5    | 3.5                   | 3.5 | 3.5 | 3.0                  | 3.0 | 2.0 | 2.0                                 |

\*Sodium Hexametaphosphate.

\*\*Sulfamic Acid required to lower pH after the additive added to A/T liquor.

## Summary of Results

The change in the dyed shade was reduced (went more to the blue side) when the sequestering agent was used.

Light induced yellowing was improved between 1 to 55 1 gray scale unit at 20 AFU using the sequestering agent. No further improvement was noted going from the low to the high concentration. There also appeared to be more of an improvement (or fading) of the yellowing in going from 20 to 40 AFU's when the sequestering agent was included.

Yellowing upon exposure to ozone was also minimized when the sequestering agent was included. Only a slight reduction in the yellowing upon exposure to nitrogen dioxide was observed.

There was no impact on staining, but a slight reduction in the Interatex N analyzed on carpet level was observed when the sequestering agent was used.

TABLE XXXII

ADDITION OF SEQUESTERING AGENTS TO  
INHIBIT LIGHT INDUCED YELLOWING  
STAINING DATA

| Sample | I.D. | A/T pH | Stain Rating<br>(0 = best 10 worst) |      |      |      | Shade Change* |
|--------|------|--------|-------------------------------------|------|------|------|---------------|
|        |      |        | 1                                   | 4    | 8    | 24   |               |
| 1      | —    | —      | 9.5                                 | 9.5  | 9.5  | 9.5  | —             |
| 2      | 3.0  | 0.25   | 0.25                                | 0.75 | 0.75 | 1.25 | M-N           |
| 3      | 3.3  | 0.75   | 0.75                                | 0.75 | 0.75 | 0.75 | M-N           |
| 4      | 3.2  | 0.25   | 0.75                                | 0.75 | 0.75 | 0.75 | M-N           |
| 5      | 3.7  | 0.5    | 1.0                                 | 1.25 | 1.25 | 1.25 | N             |
| 6      | 3.3  | 0.5    | 0.5                                 | 1.0  | 1.5  | 1.5  | M-N           |
| 7      | 3.0  | 0.25   | 0.75                                | 0.75 | 0.75 | 0.75 | N             |
| 8      | 3.3  | 0.5    | 1.0                                 | 1.0  | 1.0  | 1.0  | N             |
| 9      | 3.6  | 0.25   | 0.5                                 | 1.0  | 1.0  | 1.0  | N             |

\*M = moderate N = none

## EXAMPLE 8

Method for Exhausting Ammonium Thiocyanate Onto  
Dyed Nylon Fiber to Improve its Resistance to  
Oxidizing Agents

## Description of the Embodiment

Dyed carpet fiber, especially that made from nylon, whether or not it is treated with a sulfonated aromatic condensate or other treatments, is susceptible to significant color fading due to exposure to ozone, benzoyl peroxide and products containing chlorine. The problem was lessened to some extent when the dye industry changed over to acid dyes from disperse dyes. Acid dyes were less able to migrate and be destroyed by ozone because they were electronically bound to the nylon. However, the use of acid dyes did not eliminate these color fastness problems.

There are many antioxidants and antiozonants available on the market. These products are usually aromatic and contain amine or sulfur functionalities. These products have several disadvantages: aromatics usually yellow the fiber upon further heat treatment, and the amines and sulfur functionalities cause a reduction in nylon lightfastness. Also, these chemistries probably act as sacrificial agents and it has been difficult to apply enough onto the fiber to have long term benefit.

The thiocyanates, such as ammonium thiocyanate, are antiozonants that are well known. The cation of the thiocyanate may be ammonium, sodium, potassium, zinc, copper, ferrous, ferric, methyl or phenyl. They had the additional advantage over the other antioxidants in that they do not reduce lightfastness. However, it has not been economically possible to apply enough of the thiocyanate during dyeing to have long term effectiveness as it is also a sacrificial agent. (Ammonium thiocyanate also appears to agglomerate the dye molecules which also improves ozone fastness.)

In order to apply ammonium thiocyanate economically, it is necessary to devise a process in which it essentially exhausts onto the fiber. At pH=7 and 212° F. (100° C.) (normal dyeing conditions), the ammonium thiocyanate will not exhaust onto the fiber as it is water soluble and not very substantive to nylon. However, it has been found that at acidic pH's, especially at about pH 1.5 to pH 5, the ammonium thiocyanate will exhaust onto the nylon.

## Comparison of Various Thiocyanates

A comparison was made of the performance of several organic and inorganic thiocyanate compounds which had been aftertreated onto fluorocarbon treated nylon carpet fiber knitted into sleeves at pH=2, 140° F. (60° C.), 20:1 liquor:goods and 20 minutes. No dyes were added. The following thiocyanates were evaluated:

| Added as Received, % | Thiocyanate                        | Activity % |
|----------------------|------------------------------------|------------|
| 0.30                 | NH <sub>4</sub> SCN                | 100        |
| 0.32                 | NaSCN                              | 100        |
| 0.38                 | KSCN                               | 100        |
| 0.48                 | CuSCN                              | 100        |
| 2.57                 | CH <sub>2</sub> (SCN) <sub>2</sub> | 10         |
| 3.13                 | Ph(S)N=CCH <sub>2</sub> SCN        | 30         |

The amounts added introduced an equivalent quantity of thiocyanate concentration onto the fiber.

The ammonium, sodium and potassium thiocyanates were all equally superior to untreated nylon in resistance to ozone, benzoyl peroxide and chlorine bleach fastness. The other 15 thiocyanates were slightly more resistant to these color fade tests than the untreated nylon. The xenon lightfastness of all the samples were similar to untreated nylon except CuSCN which was more resistant and the phenyl-based thiocyanate which was much worse.

## Effect of pH

Using the same condition as above but varying pH and using only NH<sub>4</sub>SCN, the percent exhaustion of NH<sub>4</sub>SCN onto fiber was measured at the pH levels shown.

|    | pH | Exhaustion, % |
|----|----|---------------|
| 20 | 1  | 60            |
|    | 2  | 60            |
|    | 3  | 40            |
|    | 4  | 10            |
|    | 5  | 10            |
|    | 6  | 8             |
| 25 | 7  | 9             |

## Effect of Temperature

In another test at the same conditions pH 2 temperature was varied to achieve the following exhaustion levels.

|    | Temperature. |      | Exhaustion,<br>% |
|----|--------------|------|------------------|
|    | °F.          | °C.  |                  |
| 35 | 75           | 23.9 | 70               |
|    | 100          | 37.8 | 66               |
|    | 120          | 48.9 | 63               |
|    | 140          | 60.0 | 60               |
| 40 | 180          | 82.2 | 75               |
|    | 200          | 93.3 | 98               |

Thus by raising the temperature, it is expected that more complete exhaustion can be achieved at higher pH levels.

In a separate test at the same conditions but varying time, it was found that time between 5 and 50 minutes had little effect on exhaustion levels. On the other hand, increasing the concentration of NH<sub>4</sub>SCN lowers the level of exhaustion. It was also found that putting increasing amounts of NH<sub>4</sub>SCN on the fiber has only a very small effect on ozonefastness over 2,000 ppm, a little effect over 1,000 ppm, but a large effect between 0 and 1,000 ppm. It was noted that the ΔE in the standard 5-cycle AATCC ozonefastness changed from 6 at 500 ppm to only 2 at 1,000 ppm.

## DISCUSSION

The above examples are but a few of the many embodiments and variations of this invention. One skilled in the art would be able to select the proper conditions and amounts of chemical compounds for other embodiments of this invention to achieve the results desired after learning the teachings of this invention, including the Examples and the broader teachings of the Summary of the Invention above. The broader teachings are based on economic, technical and practical limitations to practice the invention. However, it may sometimes

be useful to operate outside these economic or practical limitations for special reasons.

The following discussion will describe some of the practical, economical and/or technical limitations of the parameters of the embodiments of this invention.

First, regarding the operating conditions of the continuous aftertreatment method, including two-step application methods, of this invention, the following table lists reasons for the limitations given.

| Limitation Variation                                                                     | Reason                                                                                                                                                                    |
|------------------------------------------------------------------------------------------|---------------------------------------------------------------------------------------------------------------------------------------------------------------------------|
| preheat water temp. below 140° F. (60° C.) and carpet temp. below 130° F. (54.4° C.)     | less uniform application during the following treatment and less effective or economic to heat carpet atmospheric process, water cannot be heated above the boiling point |
| preheat water temp. above 212° F. (100° C.) and carpet above 210° F. (°C.)               | less uniform, poor penetration                                                                                                                                            |
| less than 75% w.p.u.                                                                     | less uniform, poor penetration                                                                                                                                            |
| preheat step extracting to less than 30% w.p.u.                                          | less uniform, poor penetration                                                                                                                                            |
| extracting to above 190% w.p.u.                                                          | dilutes following application liquor, less effective                                                                                                                      |
| application pH below 1.5                                                                 | corrosive                                                                                                                                                                 |
| application pH above 5.5                                                                 | less effective, due to compounds of aqueous soln. penetrating too deep into fiber, at very high pH no exhaustion of compositions less effective                           |
| application less than 200% w.p.u.                                                        | carpet fabric cannot hold much more aqueous solution less effective                                                                                                       |
| application over 650% w.p.u.                                                             | uneconomical                                                                                                                                                              |
| conc. of s.a.c. less than 0.25 g/l                                                       | less effective                                                                                                                                                            |
| conc. of s.a.c. over 40 g/l                                                              | atmospheric process, water cannot be heated above the boil                                                                                                                |
| application soln. temp. under 140° F. (60° C.) and carpet temp. under 130° F. (54.4° C.) | less effective                                                                                                                                                            |
| application soln. temp. over 212° F. (100° C.) and carpet temp. over 210° F. (99° C.)    | adverse color fastness results                                                                                                                                            |
| less than 0.05% owf MgSO <sub>4</sub>                                                    | less effective                                                                                                                                                            |
| more than 0.8% owf MgSO <sub>4</sub>                                                     | uneconomical                                                                                                                                                              |
| less than 0.03% owf NH <sub>4</sub> SCN                                                  | less effective                                                                                                                                                            |
| more than 1% owf NH <sub>4</sub> SCN                                                     | uneconomical                                                                                                                                                              |
| less than 0.15% owf s.a.c.                                                               | less effective                                                                                                                                                            |
| more than 7.5% owf s.a.c.                                                                | uneconomical                                                                                                                                                              |
| more than 6 or 3 parts to parts of s.a.c. of the respective dispersing agents            | uneconomical, possible adverse chemical activity                                                                                                                          |

The following table lists reasons for limitation parameters for the two-step, batch-batch method of this invention.

| Limitation Variation                              | Reason                                                                                                                                                        |
|---------------------------------------------------|---------------------------------------------------------------------------------------------------------------------------------------------------------------|
| second step pH below 1.5                          | corrosive                                                                                                                                                     |
| second step pH above 5.5                          | less effective, due to compounds of aqueous soln. penetrating too deep into fiber, at very high pH no exhaustion of compositions uneconomical, takes too long |
| second step temp. below 110° F. (°C.)             | less effective, due to compounds of aqueous soln. penetrating too deep into fiber                                                                             |
| second step temp. above 195° F. (°C.)             | less uniform, poor wetting and penetration                                                                                                                    |
| first & second step liquor: fabric ratio below 10 |                                                                                                                                                               |

-continued

| Limitation Variation                                                                                                                                                    | Reason                                                                                         |
|-------------------------------------------------------------------------------------------------------------------------------------------------------------------------|------------------------------------------------------------------------------------------------|
| first & second step liquor: fabric ratio above 100                                                                                                                      | uneconomical                                                                                   |
| first step temp. below 158° F. (70° C.)                                                                                                                                 | uneconomical, nonuniform application, takes too long                                           |
| first step temp. above 212° F. (100° C.)                                                                                                                                | atmospheric process, water cannot be heated above the boil                                     |
| 10 first step treating time less than 15 minutes                                                                                                                        | blotches and streaks, nonuniform                                                               |
| first step treating time over 90 minutes                                                                                                                                | uneconomical                                                                                   |
| second step treating time under 5 minutes                                                                                                                               | nonuniform application                                                                         |
| 15 less than 0.05% owf fluorocarbon on pretreated fabric over 0.4% owf fluorocarbon on pretreated fabric below 0.25% of MgSO <sub>4</sub> over 4% owf MgSO <sub>4</sub> | does not provide anti-soiling effect                                                           |
| 20 below 0.03% owf NH <sub>4</sub> SCN above 1% owf NH <sub>4</sub> SCN below 0.15% owf s.a.c. above 7.5% owf s.a.c.                                                    | ineffective poor lightfastness, uneconomical, poor dyeing, shade changes                       |
| 25 below 0.03% owf NH <sub>4</sub> SCN above 1% owf NH <sub>4</sub> SCN below 0.15% owf s.a.c. above 7.5% owf s.a.c.                                                    | ineffective uneconomical ineffective fabric discolors, fabric stiff, poor dye yield, yellowing |

The benefits of the best mode of this invention using Composition 1 in a two-step, continuous-continuous process as described above in Example 1 are given below. Most or some of the individual benefits given are also achieved by the other embodiments of this invention.

30 35 40 45 50 improved stain resistance, particularly for carpet fabric of high ICP nylon fiber, substantially eliminates light induced yellowing of sulfonated aromatic condensate treated fiber, reduces NO<sub>2</sub> yellowing of sulfonated aromatic condensate treated fiber, improves resistance of dye on sulfonated aromatic condensate treated fiber to fading from ozone and oxidation by benzoyl peroxide, improves penetration of sulfonated aromatic condensate and treatment chemicals into the carpet fabric, including the base or backing, does not significantly impact the soil resistance of the fluorocarbon treatment on the fiber of the carpet fabric, improves durability of the sulfonated aromatic condensate and treatment chemicals to steam cleaning with high pH detergents.

We claim:

1. A two-step method to continuously treat dyed nylon carpet fabric with a sulfonated aromatic condensate to impart resistance to staining comprising:  
55 adding a first portion of said sulfonated aromatic condensate during dyeing of said carpet fabric in an amount of at least 0.05% sulfonated aromatic condensate based on the weight of the nylon fiber in said carpet fabric,  
60 preheating said dyed carpet fabric with water at a temperature between about 140° and 212° F. (60° and 100° C.) to a wet pick-up of above about 75% by weight, and a carpet temperature of between about 130° and 210° F. (54.4° and 99° C.), then extracting said water from said carpet fabric to a wet pick-up of between about 30 to 190% by weight, then

applying an aqueous solution of a second portion of said sulfonated aromatic condensate, in an amount of at least 0.05% sulfonated aromatic condensate based on the weight of the nylon fiber in said carpet fabric, to said carpet fabric at a pH of between about 1.5 to 5.5, at a concentration of between about 0.25 and 40 grams of solids of said condensate per liter of aqueous solution, at a wet pick-up of between 200 and 650% by weight, at an aqueous solution liquor temperature of between about 140° 10 and 212° F. (60° and 100° C.), to achieve a carpet fabric temperature between about 130° and 210° F. (54.4° and 99° C.), then

holding said carpet in said aqueous solution for between about 0.5 to 90 seconds at a temperature 15 above 130° F. (54.4° C.), so that the portion of sulfonated aromatic condensate added during dyeing and the portion of sulfonated aromatic condensate added after dyeing combined make an amount effective to impart to said carpet fabric resistance 20 to staining.

2. The method of claim 1 wherein an electrolyte having a divalent cation is also added to the aqueous solution during said dyeing in an amount of at least 0.03% based on weight of the nylon fiber so that stain 25 resistance of the nylon fiber in the carpet fabric is enhanced and durability to steam cleaning of said stain resistance is enhanced, wherein the electrolyte is magnesium or ferrous sulfate or phosphate.

3. The method of claim 2 wherein the electrolyte is 30 magnesium sulfate.

4. The method of claim 1 wherein between about 0.05% to 0.5% on the weight of the fiber is added to the aqueous solution during dyeing and an additional 0.05% to 7.5% on the weight of the fiber of sulfonated aromatic condensate is added to the aqueous solution of 35 said second portion.

5. The method of claim 4 wherein 0.03 to 1% on the weight of the fiber of magnesium sulfate is added to the dyebath and 0.05 to 1% on the weight of the fiber of 40

magnesium sulfate is added to said aqueous solution of said second portion.

6. A method to dye and treat, in two batch steps, nylon carpet fabric to impart resistance to staining comprising

dyeing, in a first step, the undyed carpet fabric in a dye bathe liquor in the presence of a first portion of a sulfonated aromatic condensate in an amount of at least 0.05% sulfonated aromatic condensate based on the weight of the nylon fiber in said carpet fabric in an aqueous solution at an elevated temperature, then

removing the dye bath liquor from the dyed carpet fabric, then

rinsing the dyed carpet fabric, then

applying, in the second step, a second portion of a sulfonated aromatic condensate in an amount of at least 0.05% sulfonated aromatic condensate based on the weight of the nylon fiber in said carpet fabric in an aqueous solution to said dyed carpet fabric, at a pH of between about 1.5 to 5.5 and at a liquor temperature of between about 110° to 195° F. (60° to 91° C.), so that the total said first and second portions of sulfonated aromatic condensate make an amount effective to impart to said carpet fabric resistance to staining.

7. The method of claim 6 wherein said aqueous solution of both steps also contains an electrolyte having a divalent cation in an amount of at least 0.03% based on the weight of the nylon fiber so that stain resistance of the nylon carpet fabric is enhanced and durability to steam cleaning of the stain resistance is enhanced, wherein said electrolyte is magnesium or ferrous chloride, sulfate or phosphate.

8. The method of claim 6 wherein the total amount of both portions of sulfonated aromatic condensate is present in an amount between about 0.15 and 7.5% on weight of fabric.

\* \* \* \* \*